# EUROPEAN PATENT SPECIFICATION

(11) **EP 0 483 163 B1**
(45) Date of publication and mention of the grant of the patent: **10.05.1995**
(21) Application number: 90908787.6
(22) Date of filing: 17.05.1990
(51) Int. Cl.: D21C 9/153, D21C 9/147, D21C 9/10

(54) **ENVIRONMENTALLY IMPROVED PROCESS FOR BLEACHING LIGNOCELLULOSIC MATERIALS**
UMWELTFREUNDLICHERES VERFAHREN ZUM BLEICHEN VON LIGNOCELLULOSISCHEN MATERIALIEN
PROCEDE MOINS POLLUANT DE BLANCHIMENT DE MATIERES LIGNOCELLULOSIQUES

(43) Date of publication of application: 06.05.1992
(73) Proprietor: UNION CAMP PATENT HOLDING, INC., Wilmington, DE 19801 (US)
(72) Inventor: GRIGGS, Bruce, F., Columbia, SC 29223 (US); GANDEK, Thomas, P., Trenton, NJ 08618 (US); PIKULIN, Michael, A., Bround Brook, NJ 08805 (US); ROSEN, Allen, Lawrenceville, NJ 08648 (US)
(74) Representative: DIEHL GLAESER HILTL & PARTNER
(86) International application number: US9002823
(87) International publication number: WO9118145

(56) References cited:
- DE-A- 2 845 025
- US-A- 4 216 054
- US-A- 4 278 496
- US-A- 4 619 733
- US-A- 4 806 203
- TAPPI JOURNAL, Volume 67, No. 8 (LIEBERGOTT et al) August 1984, pages 76-80
- PULP AND PAPER MAGAZINE OF CANADA, Volume 75, No. 4 (Soteland) April 1974,pages 91-96

## Description

### Field of the Invention

This invention relates to a novel, environmentally acceptable process for delignifying and bleaching lignocellulosic pulp which does not require the use of elemental chlorine and which produces a pulp of acceptable strength. Use of this process also reduces the amount of environmental pollutants.

### Background of the Invention

Wood is comprised of two main components - a fibrous carbohydrate, i.e., cellulosic portion, and a non-fibrous component. The polymeric chains forming the fibrous cellulose portion of the wood are aligned with one another and form strong associated bonds with adjacent chains. The non-fibrous portion of the wood comprises a three-dimensional polymeric material formed primarily of phenylpropane units, known as lignin. Part of the lignin is between the cellulosic fibers, bonding them into a solid mass, although a substantial portion of the lignin is also distributed within the fibers themselves.

For use in paper-making processes, wood must first be reduced to pulp. Pulp may be defined as wood fibers capable of being slurried or suspended and then deposited upon a screen to form a sheet, i.e., of paper. The methods employed to accomplish the pulping step usually involve either physical or chemical treatment of the wood, or a combination of these two treatments, to alter the wood's chemical form and to impart desired properties to the resultant product. There are thus two main types of pulping techniques, i.e., mechanical pulping and chemical pulping. In mechanical pulping, the wood is physically separated into individual fibers. In chemical pulping, the wood chips are digested with chemical solutions to solubilize a portion of the lignin and thus permit its removal. The commonly utilized chemical pulping processes are broadly classified as: (1) the soda process, (2) the sulfite process, and (3) the Kraft process, with the latter process being most commonly used and being capable of a variety of well-known modifications as described below.

The soda process is well known in the art. It employs sodium hydroxide (NaOH) as the active reagent to break down the lignin and to assist in its removal. The sulfite process is also well known in the art (see, e.g., Handbook for Pulp & Paper Technologists - Chapter 6: Sulfite Pulping (TAPPI, U.S.A.).

The Kraft process together with its numerous variations is the principle chemical process utilized in paper manufacturing. The basic Kraft process, as described in the Handbook For Pulp and Paper Technologists - Chapter 7: Kraft Pulping (TAPPI, U.S.A.), involves digesting the wood chips in an aqueous solution of sodium hydroxide (NaOH) and sodium sulfide (Na₂S). This process is highly effective in the pulping of even difficult woods such as southern softwoods, as well as the other more readily pulped species of wood such as northern hardwoods and softwoods. The Kraft process likewise generally produces a relatively high-strength pulp since its use results in a diminished attack on the cellulose component of the wood.

The modified Kraft techniques can result in even less degradation in the polymeric structure of the cellulosic fibers during pulping and therefore the strength loss in the resultant paper product is diminished as compared to that occurring with the standard Kraft process. One modified Kraft pulping process is known as "extended delignification", which is a broad term used in the art to encompass a variety of modified Kraft techniques, such as adding the pulping chemicals in a specific defined sequence, or at different locations within the digester apparatus, or at different time periods, or with a removal and reinjection of cooling liquors in a prescribed sequence, so as to more effectively remove a greater amount of lignin while reducing the severity of the pulping liquor's chemical attack on the cellulosic fibers. Another modification of the Kraft process is the Kraft-AQ process, wherein a small amount of anthraquinone is added to the Kraft pulping liquor to accelerate delignification while limiting the attack upon the cellulosic fibers which comprise the wood.

A variety of additional extended delignification techniques are known in the art and include Kamyr Modified Continuous Cooking (MCC) as described by V.A. Kortelainen and E.A. Backlund in TAPPI, vol. 68 (11), 70 (1985); Beloit Rapid Displacement Heating (RDH) as reported by R. S. Grant in TAPPI, vol. 66 (3), 120 (1983); and Sunds Cold Blow Cooking as reported by B. Pettersson and B. Ernerfeldt in Pulp and Paper, vol. 59 (11), 90 (1985).

Digestion of the wood by a Kraft or modified Kraft process results in the formation of a dark colored slurry of cellulose fibers known as "brownstock". The dark color of the brownstock is attributable to the fact that not all of the lignin has been removed during digestion and has been chemically modified in pulping to form chromophoric groups. Thus, in order to lighten the color of the brownstock pulp, i.e., to make it suitable for use as printing and writing and other white paper applications, it is necessary to continue the removal of the remaining lignin by the addition of delignifying materials and by chemically converting any residual lignin into colorless compounds by a process known as "bleaching" or "brightening".

Prior to bleaching the pulp, however, the digested material is conventionally transferred to a separate blow tank after the chemical treatments involved in the pulping process are completed. Within the blow tank, the pressure developed during the initial chemical treatment of the lignocellulosic material is relieved and the pulp material is separated into a fibrous mass. The resulting fibrous mass is then subjected to a series of washing steps to remove the combination of any residual chemicals and the soluble materials (such as the lignin) which were separated from the fibrous materials in the pulping process. Frequently, the pulp also undergoes one or more screening steps designed to separate out the larger portions of undefibered wood for special processing (recooking, mechanical grinding, etc.).

The residue obtained from the washing process, commonly referred to as black liquor, is collected, concentrated, and then incinerated in an environmentally safe manner in a recovery boiler. The technique for the collection, concentration and burning of the black liquor is conventional and is well known in the art.

The delignification and bleaching processes are conducted on the washed fibrous mass in a series of steps, using selected combinations of chemical reactants. In the prior art, various combinations of chemical treatments have been suggested. Furthermore, individual treatment steps have been rearranged in an almost limitless number of combinations and permutations. Therefore, in order to simplify the explanation of the various bleaching processes and systems, the use of letter codes is conventionally employed in combination to describe the particular chemical reactants employed and the sequence of the steps of the process.

The letter codes which will be used hereafter, where appropriate, are as follows:

Oₘ and Zₘ are modified processes according to the present invention and are described further in the Detailed Description of the Invention.

It has been conventional for many years to delignify and bleach wood pulp by using elemental chlorine. Exemplifying the bleaching of lignocellulosic pulps are the processes disclosed in, for example, US-A- 1,957,937 to Campbell et al., US-A- 2,975,169 to Cranford et al. and, US-A- 3,462,344 to Kindron et al.; and Handbook For Pulp and Paper Technologists - Chapter 11: Bleaching (§11.3) (TAPPI, USA).

However, although elemental chlorine has proven to be an effective bleaching agent, it is difficult to handle and potentially hazardous to both mill personnel and equipment. For example, the effluents from chlorine bleaching processes contain large amounts of chlorides produced as the by-product of these processes. These chlorides readily corrode processing equipment, thus requiring use of costly materials in the construction of such mills. Further, the build-up of chlorides within the mill precludes recycling the washer filtrate after a chlorination stage in a closed system operation without employing recovery systems requiring extensive, and therefore expensive, modifications. In addition, concern about the potential environmental effects of chlorinated organics in effluents, which the U.S. Environmental Protection Agency believes to be toxic to humans and animals, has caused significant changes in government requirements and permits for bleach mills which include standards that may be impossible to meet with conventional bleaching or pollution control technology.

To avoid these disadvantages, the paper industry has attempted to reduce or eliminate the use of elemental chlorine and chlorine-containing compounds from multi-stage bleaching processes for lignocellulosic pulps. Complicating these efforts is the requirement that high levels of pulp brightness are required for many of the applications for which such pulp is to be used.

In this connection, efforts have been made to develop a bleaching process in which chlorine-containing agents are replaced, for example, by oxygen for the purpose of bleaching the pulp. The use of oxygen does permit the recycling of effluent from this stage for recovery and does permit a substantial reduction in the amount of elemental chlorine used. A number of processes for bleaching and delignifying pulp with oxygen have been proposed, such as Richter US-A- 1,860,432, Grangaard et al. US-A- 2,926,114 and US-A- 3,024,158, Gaschke et al. US-A- 3,274,049, Meylan et al. US-A- 3,384,533, Watanabe US-A- 3,251,730, Rerolle et al. US-A- 3,423,282, Farley US-A- 3,661,699, Kooi US-A- 4,619,733 and P. Christensen in "Bleaching of Sulphate Pulps with Hydrogen Peroxide", Norsk Skogindustri, 268-271 (1973). Alkaline pretreatments of pulp prior to oxygen delignification are suggested by US-A- 4,806,203 to Elton.

The use of oxygen, however, is not a completely satisfactory solution to the problems encountered with elemental chlorine. Oxygen is not as selective a delignification agent as elemental chlorine, and the K No. of the pulp, using conventional oxygen delignification methods, can be reduced only a limited amount until there is a disproportionate, i.e., unacceptable, attack on the cellulosic fibers. Also, after oxygen delignification, the remaining lignin has heretofore typically been removed by chlorine bleaching methods to obtain a fully-bleached pulp, but using much reduced amounts of chlorine. However, even at such reduced chlorine concentrations, the corrosive chlorides would soon reach unacceptable concentration levels in a closed cycle operation.

To avoid the use of chlorine bleaching agents, the removal of such remaining lignin with the use of ozone in the bleaching of chemical pulp has previously been attempted. Although ozone may initially appear to be an ideal material for bleaching lignocellulosic materials, the exceptional oxidative properties of ozone and its relative high cost have heretofore limited the development of satisfactory ozone bleaching processes for lignocellulosic materials, especially southern softwoods. Ozone will readily react with lignin to effectively reduce the K No., but it will also, under most conditions, aggressively attack the carbohydrate which comprises the cellulosic fibers and substantially reduce the strength of the resulting pulp. Ozone, likewise, is extremely sensitive to process conditions such as pH with respect to its oxidative and chemical stability, and such changes can significantly alter the reactivity of ozone with respect to the lignocellulosic materials.

Since around the turn of the century, when the delignifying capabilities of ozone were first recognized, there has been substantial and continuous work by numerous persons in the field to develop a commercially suitable method using ozone in the bleaching of lignocellulosic materials. Furthermore, numerous articles and patents have been issued in this area and there have been reports of attempts at conducting ozone bleaching on a non-commercial pilot scale basis. For example, US-A- 2,466,633 to Brabender et al., describes a bleaching process wherein ozone is passed through a pulp having a moisture content (adjusted to an oven dry consistency) of between 25 and 55 per cent and a pH adjusted to the range of 4 to 7.

Other non-chlorine bleach sequences are described by S. Rothenberg, D. Robinson & D. Johnsonbaugh, "Bleaching of Oxygen Pulps with Ozone", Tappi, 182-185 (1975) - Z, ZEZ, ZP and ZPₐ(Pₐ-peroxyacetic acid); Tappi Journal, vol. 67, no. 8, August 1984, Atlanta, US; N. Liebergott et al. "Bleaching a softwood kraft pulp without chlorine compounds", pages 76-80, and N. Soteland, "Bleaching of Chemical Pulps With Oxygen and Ozone", Pulp and Paper Magazine of Canada; T153-58 (1974) - OZEP, OP and ZP.

Also, US-A- 4,196,043 to Singh discloses a multi-stage bleaching process which also attempts to eliminate the use of chlorine compounds, and includes examples specifically directed to hardwoods. It is well known to those skilled in the art that hardwoods are easier to bleach than most softwoods. This process is characterized by from one to three ozone bleaching stages and a final treatment with alkaline hydrogen peroxide, each stage being separated by an alkaline extraction. One such sequence may be described in the common shorthand nomenclature of the paper industry as ZEZEP. In accordance with this process, the effluent from each treatment stage may be collected and recycled for use in bleaching operations, preferably at an earlier stage than that from which it was obtained. This patent also provides a so-called countercurrent effluent flow.

Despite all of the research conducted in this area, no commercially feasible process for the manufacture of ozone bleached lignocellulosic pulps, especially southern softwood, has heretofore been disclosed, and numerous failures have been reported.

The present invention provides novel combinations of pulping and bleaching steps which overcome the problems encountered in the prior art as discussed herein and which essentially eliminate the discharge of chlorinated organics and minimizes color and BOD releases to produce a high grade bleached pulp in a commercially feasible manner.

### Summary of the Invention

Accordingly, it is an object of the present invention to provide a multi-stage process for delignifying and bleaching lignocellulosic pulp without the use of elemental chlorine bleaching agents to substantially reduce or eliminate pollution of the environment while optimizing the physical properties of the pulp in an energy efficient, cost effective process. The present invention can work on virtually all wood species, including the difficult-to-bleach southern U.S. softwoods.

The process of the present invention as described in claim 1 is composed of three or more steps with a number of possible variations within and between the steps. These steps can be described as follows:

A first step involves delignification of wood chips into a lignocellulosic pulp, using any one of several chemical pulping processes, followed by a washing removal of most of the dissolved organics and cooking chemicals for recycle and recovery. Usually included is a screening of the pulp to remove bundles of fibers that have not been separated in pulping. This delignification step is conducted so that, for a southern U.S. softwood, for example, pulp with a K No. in the range of about 20-24 (target of 21), a cupriethylenediamine ("CED") viscosity in the range of about 21-28, and a GE brightness in the range of about 15-25 is typically obtained. For southern U.S. hardwood, pulp with a K No. in the range of about 10-14 (target 12.5) and a CED viscosity of about 21-28 is typically obtained.

Among, but not limited to, the effective embodiments of this first step are:
a. Kraft pulping using either a continuous or batch digestion stage;
b. Continuous digestion kraft pulping with extended delignification using staged alkali addition and countercurrent final cooking;
c. Batch digestion kraft pulping with extended delignification using rapid liquor displacement and cold blowing techniques; or
d. Kraft-AQ pulping to achieve extended delignification using either a continuous or batch digestion stage.

The extended delignification techniques discussed in (b) and (c) above, may include, for example, the Kamyr MCC, the Beloit RDH and Sunds Cold Blow Cooking techniques described in the background portion of this specification. Depending upon the type of lignocellulosic material used, the soda and sulfite processes mentioned above may be used.

A second step of the process includes an oxygen delignification treatment to further remove lignin without an accompanying significant loss in cellulosic fiber strength. This would include a washing removal of the dissolved organics and alkali for recycle and recovery. Pulp screening is also performed at times after oxygen delignification.

During the oxygen delignification step, the K No. of the increased consistency pulp is decreased by at least about 45% (for O) to at least about 60% (for Oₘ) without significantly damaging the cellulose component of the pulp. Also, the ratio of K No. to viscosity of the pulp is typically decreased by at least 25%. For the softwood pulp described above using Oₘ, a K No. of about 7 to 10 and a viscosity of above about 13 is easily achieved. For hardwood pulp, a K No. of about 5 to 8 and a viscosity above about 13 is achieved after the oxygen delignification step.

Among, but not limited to, the possible embodiments to this step are:
a. Conventional oxygen delignification, comprised of an alkaline oxygen treatment of the pulp at either low, medium, or high pulp consistency (O); or
b. The preferred embodiment of an alkaline treatment at low to medium pulp consistency, i.e., less than about 10% by weight, followed by high pulp consistency oxygen treatment, i.e,. greater than about 20% by weight (Oₘ).

For pulp end uses that do not require brightnesses above about 35% GEB (often referred to as semi-bleached pulp), it is possible to use pulp that has been processed only through step 2 directly in the papermaking process.

A third step of the process include an acidic, gaseous ozone bleaching treatment (Z or Zₘ) under defined process parameters to provide a highly selective removal and bleaching of lignin with minimal degradation of cellulose. Among the process parameters are chelating agents for metal ion control, pH control, pulp particle size control, pulp consistency, ozone concentration and gas/pulp contact control. Prior to treatment with ozone, the chelating agent, for example oxalic acid, diethylenetriamine pentaacetic acid ("DTPA") or ethylene diaminetetraacetic acid ("EDTA") may be added to the pulp to substantially bind with metal ions contained therein. Further, the pH of the pulp is preferably adjusted to a range of between about 1-4 prior to the third step. This may be accomplished by adding to the pulp a sufficient quantity of an acidic material. Advantageously, the consistency of the pulp is increased to between about 35-45% by weight and the particle size of the fiber flocs are comminuted to a size of about 5 mm or less prior to the ozone delignification step. Included is a dissolved organic washing stage for recycle and recovery.

During the ozone step, the pulp is preferably maintained at ambient temperature or at least at a pulp temperature of less than about 49°C (120°F). The ozone may be provided by an ozone-containing gas which may comprise, for example, oxygen or air. When an ozone/oxygen mixture is used, the ozone concentration is preferably between about 1 and 8 percent by volume, whereas for ozone/air mixtures, an ozone concentration of between about 1 and 4 percent by volume is acceptable. Within the ozone reactor vessel, the substantially delignified pulp is advanced in a manner which subjects substantially all of the pulp particles to the ozone in a uniform fashion.

It has been found that pulps with K Nos. greater than about 10 after the second step are not suitable for this third step, because of the substantial amounts of ozone required to reduce the K No. to the desired level, which typically results in the properties of the pulp being adversely and deleteriously affected by excessive ozone degradation of the cellulose fibers of the pulp. When pulp having a K No. of less than 10 is ozonated, a lesser concentration of ozone is used, with only a minimal amount of cellulose degradation occurring. The product from this ozonation step for either the starting southern U.S. softwood or hardwood described above is a pulp having a K No. of less than about 5 and generally in the range of about 3 to 4 (target of 3.5), a viscosity of above about 10, and a GE brightness of at least 50% (typically about 54% or higher for softwood and 63% or higher for hardwood).

Among, but not limited to, the effective embodiments for this step are:
a. Treatment of the acidified pulp by countercurrent contact of ozone in an oxygen or air carrier gas; or
b. Treatment of the acidified pulp by cocurrent contact of ozone in an oxygen or air carrier gas.

An additional bleaching step may then be used to bring the pulp to a desired fully bleached state, i.e., one having GE brightness levels of about 70 to 95% using any number of possible, well recognized bleaching and extraction processes. Among, but not limited to, the effective embodiments are:
a. A conventional extraction stage with washing followed by a peroxide stage with washing; (i.e., EP);
b. Conventional alkali extraction and washing stages followed by a conventional chlorine dioxide stage with washing (i.e., ED);
c. A conventional alkali extraction and washing stage followed by a conventional chlorine dioxide stage with washing, followed by a repeat of the extraction and chlorine dioxide stages (i.e., EDED); or
d. An extraction stage, augmented with either oxygen or oxygen and peroxide, followed by a conventional chlorine dioxide stage: i.e., (Eₒ)D or (Eₒₚ)D.

The extraction stage may comprise, in a further embodiment, combining the substantially delignified pulp with an effective amount of an alkaline material in an aqueous alkaline solution for a predetermined time and at a predetermined temperature correlated to the quantity of alkaline material to solubilize a substantial portion of any lignin which remains in the pulp. Thereafter, a portion of the aqueous alkaline solution may be extracted to remove substantially all of the solubilized lignin therefrom.

Following the extraction stage, the substantially delignified pulp may be treated in the additional bleaching step to raise the GE brightness of the resultant pulp to at least about 70%. Preferred brightening agents include chlorine dioxide or a peroxide.

The (Eₒ)D, (Eₒₚ)D or EDED embodiments will achieve the highest brightness levels. For the ED embodiment, the chlorine dioxide stage filtrate cannot, without treatment, be recycled for chemical recovery because of the presence of the inorganic chlorides. Since this is the only required sewered filtrate from the process, however, dramatic reductions in effluent volume, color, COD, BOD, and chlorinated organics are achieved. Color of less than 1 kg/tonne (2 pounds per ton), BOD₅ of less than 1 kg/tonne (2 pounds per ton) and total organic chloride (TOCl) of less than 1 (2) and preferably less than 0.4 (0.8) can be achieved. It is also possible to treat the chlorine dioxide stage filtrate with a membrane filtration process which will allow essentially complete recycle. In the EP embodiment, no chlorinated materials are formed in the bleaching process and virtually all the liquid filtrates can be recycled and recovered, producing an almost effluent-free process.

### Brief Description of the Drawings

FIG. 1 is a block flow diagram of the preferred methods of this invention wherein a solid line represents pulp flow and a broken line represents effluent flow;
FIG. 2 is a schematic representation of a preferred method of the invention;
FIG. 3 is a cross-sectional drawing of a portion of an ozonation apparatus shown in Fig. 2, taken along line 3--3;
FIG. 3A is a cross-sectional drawing of a portion of a preferred ozonation apparatus shown in Fig. 2, taken along line 3--3; and
FIG. 4 is a comparison of the recycle and waste streams for a variety of pulp treatment processes.

### Detailed Description of the Invention

The present invention relates to novel methods for delignifying and bleaching pulp while minimizing the degree of attack upon the cellulosic portion of the wood, thus forming a product having acceptable strength properties for the manufacture of paper and various paper products. For convenience in understanding the improvement over the prior art offered with the use of the presently disclosed delignification and bleaching process, provided below are the definitions of several parameters involved in the various stages in any delignification/bleaching process.

### A. General Definitions

Throughout this specification, the following definitions will be used:

"Consistency" is defined as the amount of pulp fiber in a slurry, expressed as a percentage of the total weight of the oven dry fiber and water. It is sometimes also referred to as pulp concentration. The consistency of a pulp will depend upon operation of and the type of dewatering equipment used. The following definitions are based on those found in Rydholm, Pulping Processes, Interscience Publishers, 1965, pages 862-863 and TAPPI Monograph No. 27, The Bleaching of Pulp, Rapson, Ed., The Technical Association of Pulp and Paper Industry, 1963, pages 186-187.

"Low consistency" includes ranges up to 6%, usually between 3 and 5%. It is a suspension that is pumpable by an ordinary centrifugal pump and is obtainable using deckers and filters without press rolls.

"Medium consistency" is between about 6 and 20%. Fifteen percent is a dividing point within the medium-consistency range. Below 15% the consistency can be obtained by filters. This is the consistency of the pulp mat leaving a vacuum drum filter in the brownstock washing system and the bleaching system. The consistency of a slurry from a washer, either a brownstock washer or a bleaching stage washer, is 9-15%. Above about 15%, press rolls are needed for dewatering. Rydholm states that the usual range for medium consistency is 10-18%, while Rapson states it is 9-15%. The slurry is pumpable by special machinery even though it is still a coherent liquid phase at higher temperatures and under some compression.

"High consistency" is above about 20% up to about 50%. Rydholm states that the usual range is 25-35% and Rapson states that the range is from 20-35%. These consistencies are obtainable only by the use of presses. The liquid phase is completely absorbed by the fibers, and the pulp can be pumped only very short distances.

Further, in this specification "pulping" is used in its conventional sense to refer to a digestion of lignocellulosic material to form brownstock. Pulping would include, for example, Kraft, the Kraft-AQ process and forms of extended delignification.

The term "modified Kraft process" is used herein to include extended delignification and all other modified Kraft processes with the exception of the Kraft-AQ process, since this process has achieved a special status and acceptance in the art and is separately known by that name. Also, the oxygen delignification step following completion of pulping will not be considered as an extended delignification; rather, we have chosen to call it a first step of a delignification process for bleaching or brightening the pulp.

Further, there are two principal types of measurements to determine the completeness of the pulping or bleaching process, i.e., the "degree of delignification" and the "brightness" of the pulp. The degree of delignification is normally used in connection with the pulping process and the early bleaching stages. It tends to be less precise when only small amounts of lignin are present in the pulp, i.e., in the later bleaching stages. The brightness factor is normally used in connection with the bleaching process because it tends to be more precise when the pulp is lightly colored and its reflectivity is high.

There are many methods of measuring the degree of delignification but most are variations of the permanganate test. The normal permanganate test provides a permanganate or "K No." which is the number of cubic centimeters of tenth normal potassium permanganate solution consumed by one gram of oven dried pulp under specified conditions. It is determined by TAPPI Standard Test T-214.

There are also a number of methods of measuring pulp brightness. This parameter is usually a measure of reflectivity and its value is expressed as a percent of some scale. A standard method is GE brightness which is expressed as a percentage of a maximum GE brightness as determined by TAPPI Standard Method TPD-103.

Moreover, where appropriate, the letter codes described in the Background Art section will be utilized to designate the various stages of pulp treatment throughout this Detailed Description of the Invention.

### B. The Process Steps of the Invention

The values (i.e., K No., viscosity and GE brightness) obtained by use of the present pulping, delignification and bleaching process, as set forth below, demonstrate the ability of this process to enhance the degree of lignin removal from the pulp while minimizing the resultant degradation of the cellulose. After the oxygen delignification step, and prior to brightening, the pulp has been partially delignified to a K No. of about 5 to 10, preferably between about 7 to 10 for U.S. softwoods and about 5 to 7 for U.S. hardwoods. This partially delignified pulp has a viscosity of above about 10, generally more than 13 and preferably, at least 14 (for softwood pulp) or 15 (for hardwood pulp). This partially delignified material thus has good strength and suitable viscosity so that it can withstand the effects of ozone. The partially delignified pulp is subjected to ozone to further delignify the pulp, thus reducing the K No. of the pulp to about 3 to 4 for both softwoods and hardwoods while increasing the GE brightness of the pulp to at least about 50-70%. For softwood pulp, a GE brightness of about 54% or higher is typically achieved, while for hardwood pulp, values of about 63% or more are attained. Thereafter, the brightness of the pulp is further increased by an alkali extraction and an additional bleaching step using chlorine dioxide or peroxide.

For convenience in understanding the present invention therefore, Fig. 1 sets forth, in schematic form, the various stages utilized in pulping, delignifying and brightening a pulp according to the invention. As illustrated in Fig. 1, the invention comprises a multi-stage process including the steps of:
(a) pulping the lignocellulosic material whereby the pulping chemicals may be recovered and reused in a manner well-known in the art;
(b) washing the pulp to remove chemical residues from the pulping liquor together with residual lignin and usually including a screening of the pulp to remove fiber bundles that have not been separated during pulping;
(c) alkaline oxygen delignification (i.e., O or Oₘ) of the pulp;
(d) washing the partially delignified pulp obtained in step (c) above to remove dissolved organics from the oxygen treatment; optionally, screening may be done at this point, while also recycling at least a portion of the effluent from this step to a previous step;
(e) chelation and acidification of the pulp to bind metal ions and to adjust the pH to a preferred level;
(f) contacting the pulp with ozone (i.e., Z or Zₘ) to further delignify and to partially bleach this material;
(g) washing the ozonated pulp, while recycling at least a portion of the effluent from this step to a previous step;
(h) caustic extraction to remove residual lignin;
(i) washing the extracted pulp while recycling at least a portion of the effluent to a previous step;
(j) adding a second bleaching agent (i.e., D or P to brighten and bleach the pulp);
(k) washing the bleached pulp to obtain a bleached product having a GE brightness of about 70-90%; and
(l) recycling at least a portion of the effluent from the P bleaching stage to a previous step; or sewering the effluent from the D bleaching stage or, after appropriate treatment, recycling this effluent to a previous step.

### 1. Pulping

The first stage in the method of the present invention wherein procedures can be utilized which improve the amount of lignin removed from the lignocellulosic material while minimizing the amount of degradation of the cellulose, is in the pulping step. The particular pulping process used in the method of the invention is, to a large extent, dependent on the type of lignocellulosic materials and, more particularly, the type of wood which is used as a starting material. Moreover, as illustrated in Fig. 1, the pulping liquor used in chemical pulping techniques may be recovered and reused in a manner well-known in the art. This step is typically followed by washing to remove most of the dissolved organics and cooking chemicals for recycle and recovery, as well as a screening stage in which the pulp is passed through a screening apparatus to remove bundles of fibers that have not been separated in pulping.

The Kraft process is generally acceptable for use with all woods as compared to the other noted processes, as the final pulps obtained from the Kraft process have acceptable physical properties, although the brownstock pulp is also darker in color.

Depending upon the lignocellulosic starting material, the results obtained with conventional Kraft processes may be enhanced by the use of extended delignification techniques or the Kraft-AQ process. Moreover, these techniques are preferred for obtaining the greatest degree of reduction in K No. of the pulp without deleteriously affecting the strength and viscosity properties of the pulp.

When using the Kraft-AQ technique, the amount of anthraquinone in the cooking liquor should be an amount of at least about 0.01% by weight, based on the oven dried weight of the wood to be pulped, with amounts of from about 0.02 to about 0.1% generally being preferred. The inclusion of anthraquinone in the Kraft pulping process contributes significantly to the removal of the lignin without adversely affecting the desired strength characteristics of the remaining cellulose. Also, the additional cost for the anthraquinone is partially offset by the savings in cost of chemicals in the subsequent Zₘ, E and D or P steps.

Alternatively, or perhaps even additively to Kraft-AQ, is the use of techniques for extended delignification such as the Kamyr MCC, Beloit RDH and Sunds Cold Blow Methods for batch digesters. These techniques also offer the ability to remove more of the lignin during pulping without adversely affecting the desired strength characteristics of the remaining cellulose.

### 2. Oxygen Delignification

The next step in the method of the present invention concerns the portion of the bleaching process which primarily involves removal of the residual lignin from the brownstock pulp being processed. In the method of this invention, this stage comprises an oxygen delignification step. The solid materials removed in this stage are oxygenated materials which can, like the black liquor, be collected, concentrated, and then incinerated in an environmentally safe manner in a conventional recovery boiler. At least a portion of the liquid phase is recycled as illustrated in Fig. 1.

It has been found that the oxygen delignification step can be conducted in the manner which allows for the removal of increased percentages of the remaining lignin in the brownstock pulp without causing an unacceptable corresponding decrease in the viscosity of the pulp. Broadly, the process which has been identified is practiced by treating the brownstock pulp from the pulping process at low to medium consistency, as described below, with the required amount of alkali necessary for the oxygen delignification step so as to ensure uniform application of the alkali, and thereafter raising the consistency and delignifying at high consistencies. Although high consistency delignification is preferred, low or medium consistency oxygen delignification techniques may be utilized in place of high consistency delignification.

The high consistency oxygen delignification step is preferably carried out in the presence of an aqueous alkaline solution at a pulp consistency of from about 25% to about 35%, and even more preferably, at about 27%. This improved process (Oₘ) allows for the removal of at least 60% of the residual lignin from the brownstock pulp, compared to the 45-50% removable with conventional oxygen delignification steps, without the heretofore expected undesirable decrease in the relative viscosity. Because of the unique process capabilities of this modified process, it clearly constitutes the preferred oxygen process for use in the method of this invention.

The treatment step of the modified oxygen process (Oₘ) comprises substantially uniformly combining wood pulp, preferably Kraft brownstock pulp, with an aqueous alkaline solution while maintaining the consistency of the pulp at less than about 10% and preferably less than about 5% by weight. The aqueous alkaline solution is preferably present in an amount sufficient to provide from about 0.5% to about 4% active alkali by weight after thickening based upon the oven dry pulp weight of the brownstock pulp, and even more preferably about 2.5% active alkali by weight after thickening based upon the oven dry weight of the brownstock pulp.

This step uniformly distributes the aqueous alkaline solution throughout the low consistency brownstock and ensures that substantially all the brownstock fibers are exposed to a uniform application of alkaline solution. Surprisingly, the brownstock pulp treated in this manner is not substantially delignified in the treatment step, but it is more effectively delignified in the subsequent high consistency oxygen delignification step than brownstock that is treated with alkaline solutions at high consistency according to the methods conventionally employed. The localized inhomogeneities in the distribution of alkali in conventional high consistency pulp are avoided, thus eliminating attendant non-uniform oxygen delignification.

This homogeneous distribution step thus preferably comprises uniformly combining the pulp with an aqueous alkaline solution for at least about 1 minute and preferably no more than about 15 minutes. It is believed that treatment times of less than about 1 minute will not generally provide sufficient time to attain substantially uniform distribution, whereas treatment times in excess of about 15 minutes are not expected to produce substantial further benefit.

Moreover, the preferred alkaline treatment of pulp according to the present invention may be carried out over a wide range of temperature conditions. According to a preferred practice, the treatment step is carried out at a temperature of from about room temperature to about 65°C (150°F), with temperatures ranging from about 33°C (90°F to about 65°C (150°F) being even more preferred. Atmospheric pressure or elevated pressure may be employed. The treatment step is completed when the aqueous alkaline solution is substantially uniformly distributed throughout the low consistency pulp. The amount of aqueous alkaline solution present in the treatment step can vary greatly according to the particular process parameters of the delignification reaction. The amount of the alkaline solution effective for the purpose of the present invention will depend primarily upon the extent of delignification desired in the oxygen bleaching step and the strength of the particular solution being used. The aqueous alkaline solutions preferably used comprise a sodium hydroxide solution having a concentration of from about 20 to about 120 g/l. This solution is mixed with the low consistency pulp, so that the overall mixture has a concentration of alkaline material of between about 6.5 and 13.5 g/l, and preferably around 9 g/l. Thus, for a 5 to 15 minute treatment of a 3 to 5 percent consistency pulp at temperatures between 49 and 65°C (120 to 150°F) at these concentrations of alkaline material, a uniform distribution of such alkaline material is obtained throughout the pulp.

According to a preferred embodiment of the present invention, an aqueous sodium hydroxide solution is added to the low consistency pulp in an amount sufficient to provide from about 15% to about 30% by weight of sodium hydroxide based on dry pulp weight. Other alkaline sources having an equivalent sodium hydroxide content, such as oxidized white liquor from the conventional Kraft recovery and regeneration cycle, may also be employed.

Following the low consistency caustic treatment step described above, the consistency of the treated pulp is increased to greater than about 20%, preferably from about 25% to about 35%. Several methods are available and well known in the art for increasing the consistency of the pulp, such as pressing the wood pulp to remove liquid therefrom.

Thereafter, oxygen delignification is conducted on the high consistency pulp. Methods are available and well known in the art for dissolving gaseous oxygen into the liquid phase of high consistency pulp to affect delignification thereof. It is contemplated that any of these well known methods are adaptable for use according to the present invention. It is preferred, however, that oxygen delignification according to the present invention comprise introducing gaseous oxygen at about 551600 to 689500 N/m² (80 to about 100 psig) into the liquid phase of the high consistency pulp while maintaining the temperature of the pulp between about 90°C and 130°C. The average contact time between the high consistency pulp and the gaseous oxygen is preferably from about 20 minutes to about 60 minutes.

By following the preferred process according to the present invention, it is possible to obtain a reduction in K No. for the pulp after the oxygen delignification step of at least about 60% with essentially no damage to the cellulose portion of the pulp. By comparison, conventional oxygen delignification can only achieve reductions in K No. of about 50% before degradation of cellulose occurs. Thus, the present preferred process unexpectedly provides an increase of at least 20% in delignification compared to prior art delignification processes: i.e., from 50% to at least about 60% reduction of the K No. for the incoming pulp. Reductions of 70% and more can even be achieved with minimal cellulose degradation. The avoidance of deterioration of the cellulose component of the pulp is evident by the minimal change in viscosity of pulp which is treated in accordance with the present invention.

Upon entering the oxygen delignification step, pulp K Nos. for the particular pulp range from about 10-26 depending upon the type of wood (e.g., for Kraft pulping, about 10-14, target 12.5 for hardwood and about 20-24, target 21, for softwood), while after oxygen delignification, the K No. is generally in the range of about 5-10.

A processing scheme for carrying out the method of the present invention is depicted in schematic form in Fig. 2. The steps depicted therein represent a preferred operating system that tends to maximize certain benefits of the present invention. Wood chips 2 are introduced into a digester 4 where they are cooked in a liquor such as a liquor of sodium hydroxide and sodium sulfide. The cooking unit 4 produces a Kraft brownstock 8 and a black liquor 6 containing the reaction products of lignin solubilization. The brownstock is treated in washing units comprising, preferably, blow tank 10 and washer 12 where residual liquor contained in the pulp is removed. Many methods are available and well known in the art for washing brownstock, such as diffusion washing, rotary pressure washing, horizontal belt filtering, and dilution/extraction. These methods are all within the scope of the present invention. Also, screening of brownstock is often done either before or after the washing steps in order to remove larger portions of undefibered wood for special processing.

The washed brownstock is introduced into a treatment unit 14 where it is treated with an alkaline solution and maintained at a consistency of less than about 10% and preferably less than about 5%. The process of the present invention preferably includes means for introducing make-up caustic 16 into the treatment stage to maintain the desired caustic application level. The treated pulp 18 is forwarded to a thickening unit 20 where the consistency of the pulp is increased, by pressing for example, to at least about 20% by weight and preferably to about 25% to about 35%. The liquid 22 removed from the thickening unit 20 is preferably returned to washing unit 12 for further use. The high consistency "pressed" brownstock 24 produced in the thickening unit 20 is forwarded to the oxygen delignification reactor vessel 26 where it is contacted with gaseous oxygen 28. The delignified brownstock 30 is preferably forwarded through blow tank 32 and then to a second washing unit 34 wherein the pulp is washed with water to remove any dissolved organics and to produce high quality, low color pulp 36. At least a portion of the effluent 38 from this washing step is preferably returned to washing unit 12 for use therein. The effluent 13 from washing unit 12 may be recycled alone or optionally with all or a portion of effluent 38, to either the blow tank 10 or ultimately black liquor line 6. Additionally, the partially delignified pulp obtained after oxygen delignification may be screened to remove fiber bundles from the pulp that have not separated for further treatment such as mechanical grinding. From here, pulp 36 could be sent to subsequent bleaching stages to produce a fully bleached product.

In a particularly preferred method of the present invention as shown in Fig. 2, in order to successfully utilize ozone bleaching, Kraft pulping of the wood may be carried out, followed by the modified low-consistency alkali treatment/high consistency oxygen delignification procedure (Oₘ) described above. For softwoods, as noted above, this combination results in a pulp with a K No. of about 8 to 10, preferably 9, and a viscosity of greater than about 13 to 14. Alternatively, it is possible to subject the wood to Kraft AQ pulping followed by a conventional oxygen delignification step (i.e., 0, high consistency alkaline treatment followed by high consistency oxygen delignification) to achieve a pulp having similar characteristics. In place of Kraft AQ pulping, it is also possible to use extended delignification processes, followed by a standard oxygen delignification step to achieve pulp with the desired properties. Also useful, although less preferred due to increased costs or process steps, is the combination of Kraft pulping with extended delignification techniques such as Kamyr MCC, Beloit RDH or the Sunds Cold Blow Cooking process, as described in the Background Art section of this specification, followed by conventional oxygen delignification.

Any of a wide variety of pulping and oxygen delignification steps can be used in combination as long as they achieve the above K No. and viscosity values prior to the ozone step.

Conventional Kraft pulping followed by conventional oxygen delignification is generally not acceptable in this invention, except for certain hardwoods such as aspen which are relatively easy to delignify and bleach, since for a given wood species the combination of these conventional techniques normally requires the use of the greatest amount of ozone in the ozonation step with concomitant greater cellulose degradation.

By use of the present invention, the ozone consumption may be reduced by using a number of alternate routes, such as standard kraft cooking followed by a modified oxygen delignification step (Oₘ), or modified kraft pulping with extended delignification (such as Kamyr MCC, Beloit RDH or Sunds Cold Blow) followed by a conventional oxygen delignification step (O), or by Kraft AQ cooking followed by a conventional oxygen delignification step (O) as discussed above. An even greater reduction in ozone consumption will be achieved both with the use of modified Kraft pulping with extended delignification (Kamyr MCC, Beloit RDH or Sunds Cold Blow) followed by a modified oxygen delignification step (Oₘ), or alternately when a Kraft AQ cooking process with extended delignification (Kamyr MCC, Beloit RDH or Sunds Cold Blow) is followed by a conventional oxygen delignification step (O). Using all of these techniques together in one process, i.e., Kraft AQ cooking modified by extended delignification (Kamyr MCC, Beloit RDH or Sunds Cold Blow), followed by a modified oxygen delignification step (Oₘ), reduces the amount of ozone consumed even further. Reduction in the amount of ozone consumed generally permits the viscosity of the pulp to be maintained at acceptable levels.

The advantages of using the modified high consistency oxygen delignification bleaching step (Oₘ) described above are clearly illustrated by comparison of the K Nos. and viscosities obtained using southern softwoods to related processes under otherwise substantially identical process conditions. Using a conventional Kraft pulping procedure and conventional high consistency oxygen delignification bleaching, the resulting pulps obtained will typically have a K No. of about 12 to 14 and a viscosity of about 15. This K No. is too large to permit later delignification using the ozone stage of the present invention. However, the use of conventional Kraft pulping with the modified high consistency oxygen bleaching surprisingly results in a pulp having a K No. of less than about 9, while the viscosity of the pulp is above about 12 to 14. This preferred pulp K No. permits utilization of the ozone delignification bleaching stage of the invention.

### 3. The Ozone Step

The next step in the method of this invention is ozone delignification and bleaching of the oxygen-delignified brownstock pulp. This ozonation takes place in an ozone reactor which is described below in detail and illustrated in Figs. 2, 3 and 3A. Prior to treatment of the pulp with the ozone, the pulp is conditioned so as to ensure the most effective selective delignification of the pulp and to minimize the chemical attack of the ozone on the cellulose. The incoming pulp 36 is directed into a mixing chest 40, where it is diluted to a low consistency. An acid 42 such as sulfuric acid, formic acid, acetic acid or the like, is added to the low consistency pulp to decrease the pH of the pulp in mixing chest 40 to the range of about 1 to 4 and preferably between 2 and 3. The pH is adjusted as described above since it is known that the relative effectiveness of ozone bleaching of pulps is dependent upon the pH of the pulp mixture. Lower pH values do not appear to have any beneficial effect on the further processing of the pulp, whereas increasing the pH to above about 4 to 5 causes a decrease in viscosity and an increase in ozone consumption.

The acidified pulp is treated with chelating agent 44 to complex any metals or metal salts which may be present in the pulp. This chelating step is used to render such metals non-reactive or harmless in the ozone reactor so that they will not cause breakdown of the ozone, thus decreasing the efficiency of the lignin removal and also reducing the viscosity of the cellulose.

Chelating agents are known per se and include, for example, polycarboxylate and polycarboxylate derivatives such as the di-, tri-, and tetra-carboxylates, amides, and the like. Preferred chelating agents for this ozone treatment, for reasons of cost and efficiency, include DTPA, EDTA and oxalic acid. Amounts of these chelating agents ranging from about 0.1% to about 0.2% by weight of oven dry pulp are generally effective, although additional amounts may be needed when high metal ion concentrations are present.

The effectiveness of the ozone bleaching process is controlled by a number of inter-related process parameters, including the pH level and the amount of metal salts in the pulp as discussed above. Another very important parameter is the consistency of the pulp during the ozone bleaching process. The pulp which is to be bleached must contain sufficient water so that the water exists as a continuous phase through the individual fibers, that is, the fiber should be sufficiently saturated with water. The water in the fiber allows the transfer of the ozone from the gaseous ozone atmosphere to both treat the outer surface of the fibers, and possibly more importantly, for the ozone to be transferred via the water phase to the less accessible interior portion of the individual fibers and thereby provide more complete removal of lignin from the fibers. The consistency, on the other hand, should not be so low that the ozone is diluted and tends to chemically break down rather than bleach the pulp.

The preferred range of consistency, especially for southern U.S. softwood, has been found to be between about 28% and about 50%, with the optimum results being obtained at between about 38% and about 45%. Within the above ranges, preferred results are obtained as indicated by the relative amount of delignification, the relatively low amount of degradation of the cellulose, and the noticeable increase in the brightness of the treated pulps.

The reaction temperature at which the ozone bleaching is conducted is likewise an important controlling factor in the process of the present invention. The ozone step can be effectively conducted at temperatures up to a certain critical temperature, at which the reaction commences to cause excessive degradation of the cellulose. This critical temperature will vary significantly depending upon the particular type of wood employed to form the pulp and the history of the prior treatment of the pulp. The maximum temperature of the pulp fiber at which the reaction should be conducted should not exceed the temperature at which excessive degradation of the cellulose occurs, which with southern U.S. softwood is a maximum of about 49-65°C (120°F - 150°F).

The ozone gas which is used in the bleaching process may be employed as a mixture of ozone with oxygen and/or an inert gas, or can be employed as a mixture of ozone with air. The amount of ozone which can satisfactorily be incorporated into the treatment gases is limited by the stability of the ozone in the gas mixture. Ozone gas mixtures which typically contain about 1-8% by weight of ozone in an ozone/oxygen mixture, or about 1-4% ozone in an ozone/air mixture, are suitable for use in this invention. The higher concentration of ozone in the ozone gas mixture allows for the use of relatively smaller size reactors and shorter reaction time to treat equivalent amounts of pulp, thereby lessening the capital cost required for the equipment. However, ozone gas mixtures containing lower amounts of ozone tend to be less expensive to produce and may reduce operating costs.

A further controlling factor is the relative weight of the ozone used to bleach a given weight of the pulp. This amount is determined, at least in part, by the amount of lignin which is to be removed during the ozone bleaching process, balanced against the relative amount of degradation of the cellulose which can be tolerated during ozone bleaching. In accordance with the preferred method of this invention, an amount of ozone is used which will react with about 50% to 70% of the lignin present in the pulp. The entire amount of lignin in the pulp is not removed in the ozone bleaching step as evidenced by the K No. of about 3 to 4 obtained after this step, because the absence of all lignin in the reaction zone would result in the ozone reacting excessively with the cellulose to substantially decrease the degree of polymerization of the cellulose. In the preferred method of this invention, the amount of ozone added, based on the oven dried weight of the pulp, typically is about from 0.2% to about 1% to reach the lignin levels of a 3-4 K No. Higher amounts may be required if significant quantities of dissolved solids are present in the system.

The time of the reaction used for the ozone bleaching step is determined by the desired rate of completion of the ozone bleaching reaction as indicated by complete or substantially complete consumption of the ozone which is utilized. This time will vary depending upon the concentration of the ozone in the ozone gas mixture, with relatively more concentrated ozone mixtures reacting more quickly, and the relative amount of lignin which it is desired to remove. The time required is preferably less than two minutes, but the procedure may take substantially longer depending on other reaction parameters.

An important feature of the invention is that the pulp is bleached uniformly. This feature is obtained in part, by comminution of the pulp into discrete floc particles of a size which is of a sufficiently small diameter and of a sufficiently low bulk density so that the ozone gas mixture will completely penetrate a majority of the fiber flocs, i.e., which comprise agglomerations of fibers. During comminution it is not feasible to completely separate the pulp fibers into distinct fibers. In general, the floc particles resulting from comminution have a relatively compacted central core surrounded by a plurality of outwardly extending fibers. For purposes of this invention, the floc particle size is determined by measuring what was determined to be the smallest diameter of this relatively unfluffed central core.

Bleaching uniformity is to a large extent also dependent on certain of the other process parameters, but it has been found that if the floc particle size is limited to a maximum of 5mm, and preferably even less --for example, 3mm-- that uniform treatment of a substantial majority of these particles can readily be achieved, as evidenced by observation of an insignificant number of darker underbleached floc centers. Where the floc particle size was greater than about 5mm, bleaching was non-uniform, as evidenced by a majority of darker unbleached floc centers. Therefore it is important to achieve sufficient comminution so that a majority of the flocs measure below an average of about 5 mm for uniform ozone treatment thereof.

A still further important process parameter is that during the ozone bleaching process the particles to be bleached should be exposed to the ozone bleaching mixture by mixing so as to allow access of the ozone gas mixture to all surfaces of the flocs and equal access of the ozone gas mixture to all flocs. The mixing of the pulp in the ozone gas mixture gives superior results with regard to uniformity as compared to the results obtained with a static bed of flocs wherein some of the flocs are isolated from the ozone gas relative to other flocs and thereby bleached less than other flocs.

The movement of the flocs so as to expose them to the ozone gas mixture causes uniform treatment of the flocs with respect to each other. This treatment results in the desired amount of lignin being removed uniformly from the pulp without excessive deterioration of the cellulose in the fibers which comprise the flocs. The control of the ozone treatment in accordance with this invention by use of a controlled particle size and by turbulent movement during ozone treatment has been found to result in a final pulp typically having less than about a 5% variation in GE brightness, K No. and viscosity. In comparison, if the treatment is non-uniform, as typically occurs in static bed reactors (that is, reactors wherein the particles are not agitated during ozone treatment), some portions of the bed are substantially over-bleached while other portions remain relatively unreacted because the flow of the ozone gas mixture through the static bed reactor is not uniform.

Treating pulp at high consistencies with ozone without paying particular attention to the comminution of the pulp fibers or to the proper contact between the individual fibers and the reactant gas stream invariably results in a non-uniform ozone bleaching of the fibers. The present application designates such a non-uniform ozone treatment with the letter "Z". The use of a modified ozone technique according to the present invention, as discussed above, in which the fibers are comminuted to a size of about 5 mm or less and are properly and uniformly contacted with the ozone gas stream, has been designated herein as "Zₘ".

Pulp exiting the ozone reactor has a GE brightness of about at least 50 percent and generally around 50 to 70 percent, with hardwoods usually being above about 55 percent. The pulp (for hardwoods or softwoods) also has a K No. of between about 3 and 4 (target of 3.5), which is entirely satisfactory for pulp at this stage of the process.

An apparatus which is especially suitable for ozone bleaching in accordance with the present invention is illustrated in Figs. 2, 3 and 3A. As described above, washed pulp 36 is directed to mixing chest 40 where it is treated with an acid 42 and a chelating agent 44. The acidified, chelated low-consistency pulp 46 is introduced into thickening unit 48 for removing excess liquid 50 from the pulp, such as a twin roll press wherein the consistency of the pulp is raised to the desired level. At least a portion of this excess liquid 50 may be recycled to mixing chest 40, with a remaining portion being directed to blow tank 32. The resulting high consistency pulp 52 is then passed through screw feeder 54 which acts as a gas seal for the ozone gas and thereafter through a comminuting unit 56, such as a fluffer, where the pulp is comminuted to pulp fiber flocs 60 of a pre-determined size which, as noted above, should measure about 5 mm or less in size. The comminuted particles are then introduced into a dynamic ozone reaction chamber 58 which, as illustrated, is a conveyor 62 powered by motor 64. Conveyor 62 is specifically designed for mixing and transporting the pulp particles 60 so as to allow the entire surface of the particles to become exposed to the ozone gas mixture 66 during movement of the pulp. As further shown in Fig. 2, pulp fiber flocs 60 after treatment are allowed to fall into dilution tank 68.

Fig. 3 is a cross-sectional view through ozone reactor 58 illustrating the arrangement of the pulp particles 60 as they are carried through the reactor by conveyor 62. Fig. 3A is a cross-sectional view of a preferred conveyor utilizing a paddle-like arrangement to move the comminuted particles through reaction chamber 58.

The process in Fig. 2 shows the pulp being treated with ozone cocurrently with the ozone-gas mixture. Alternately, however the portion of the pulp which has been bleached to the greatest extent may initially be contacted with the newly introduced ozone mixture containing the maximum amount of ozone by passing the ozone-containing gas in a direction counter-current to the flow of pulp 60. The pulp entering the reactor has the highest lignin content and initially contacts the exiting, nearly exhausted ozone mixture, thereby providing the optimum chance to consume virtually all of the ozone. This is an efficient method for stripping ozone from the ozone/oxygen or ozone/air mixture.

When the ozone 66 is contacted with the pulp in a cocurrent manner, as shown in Fig. 2, the remaining spent ozone gas 70 can be recovered from dilution tank 68. In tank 68, dilution water 72, which also serves as an ozone gas seal, is added to reduce the consistency of the pulp to a low level to facilitate movement of the bleached pulp 74 through the subsequent process steps.

The spent ozone gas 70 from dilution tank 68 is directed to a carrier gas pretreatment stage 76 where a carrier gas 78 of oxygen or air is added. This mixture 80 is directed to ozone generator 82 where the appropriate amount of ozone is generated to obtain the desired concentration. The proper ozone/air mixture 66 is then directed to ozone reactor 58 for delignification and bleaching of the pulp.

After completion of the ozone bleaching step, the substantially delignified pulp 74 is again thoroughly washed in washer 84 as shown in Fig. 2 and at least a portion of the water 86 which is recovered is recycled to washing unit 34 of the process, thereby producing major environmental benefits from the elimination of sewered liquid.

The bleached low consistency pulp 74 after ozonation will have a reduced amount of lignin, and therefore, a lower K No. and an acceptable viscosity. The exact values for the K No. and the viscosity which are obtained are dependent upon the particular processing to which the pulp has been subjected. For example, a southern U.S. softwood pulp which is pulped with a conventional Kraft method, initially delignified by modified high consistency oxygen delignification (Oₘ), and subsequently further delignified with ozone, preferably by a modified uniform ozone treatment (Zₘ), will typically have a K No. of about 3-4 and a viscosity of about 10. Southern U.S. softwood pulp which is subjected to Kraft AQ pulping and then to modified high consistency oxygen bleaching (Oₘ) and modified uniform ozone treatment (Zₘ) will typically have a K No. of about 2 and a viscosity of greater than about 12.

The resulting pulp 74 will be noticeably brighter than the starting pulp. For example, southern softwood, after the pulping process, has a GE brightness of about 15% to 25%; after the oxygen bleaching process, a GE brightness of about 25% to 45%; and after the ozone bleaching process, a GE brightness of about 50% to 70%.

### 4. Alkaline Extraction

The washed pulp 88 from the ozone stage is then combined with a sufficient amount of alkaline material 90 in extraction vessel 92 to effect extraction. Thus, pulp 88 is subjected to an aqueous alkaline solution for a predetermined time and at a predetermined temperature correlated to the quantity of alkaline material to solubilize a substantial portion of any lignin which remains in the pulp, in vessel 92. This extraction process also increases the brightness of the pulp, typically by about 2 GE brightness points. Thereafter, the alkali treated pulp 94 is directed to washing unit 96, the aqueous alkaline solution is washed from the pulp so as to remove substantially all of the solubilized lignin from the pulp, thus forming a substantially lignin-free pulp. This step is well known to those skilled in the art and no further comment is deemed necessary here. The examples illustrate the preferred extraction parameters for this step of the process. At least a portion of the alkaline solution 98 which is recovered is recycled to washing unit 84. Again, major environmental benefits are achieved from the elimination of sewering of this solution.

In some cases, particularly where higher final brightnesses are targeted, the extraction step can be augmented by incorporating an oxygen treatment within the caustic extraction step (Eₒ). This alternative, also well known to those skilled in the art, requires no further comment here.

### 5. Additional Bleaching Stages

For most papermaking purposes, a final brightness in the range of 50 to 65 is unsatisfactory. Accordingly, in order to further raise the GE brightness to the more desirable range of about 70 to 95%, the pulp is subjected to brightening bleaching, which is primarily intended to convert the chromophoric groups on the lignin remaining in the pulp into a colorless state.

After extracting and rewashing the pulp, the brightening bleaching of the ozone-bleached and extracted pulp can be performed using a variety of materials. As illustrated in Fig. 2, the washed pulp 100 is combined with the chosen bleaching agent 102 in bleaching vessel 104. The preferred bleaching agent is chlorine dioxide or peroxide. After bleaching, the pulp 106 is washed with water 114 in washing unit 108 and the effluent is either recycled 110 or sewered 112. When recycled, at least a portion of wash water stream 110 is directed to washing unit 96. The resultant bleached pulp 116 may then be collected and used in a variety of applications.

One of the principal materials which has heretofore been used, and which is generally highly effective, is chlorine dioxide (D) (see Fig. 1). In accordance with the invention, an appropriate amount of chlorine dioxide enables high-strength pulps having a GE brightness value greater than about 80% to be obtained. Since the pulps entering the chlorine dioxide stage are relatively low in lignin, the chlorine dioxide brightening bleaching can be carried out in the presence of only from about 0.25% to about 1% of chlorine dioxide based on the oven dry weight of the pulp.

The chlorine dioxide which is utilized in the brightening process should preferably be prepared by a process which is free from elemental chlorine. Alternatively, however, and less preferably, chlorine dioxide which does contain a minor amount of elemental chlorine can be used without any substantial increase in the relative amount of undesirable pollutants because of the relatively low amount of lignin present in the ozone-bleached pulp. The effluent from the final bleaching step of this invention when using chlorine dioxide is exceptionally low and can be discharged safely as shown in Fig. 2.

If sewering of the effluent from the final chlorine dioxide bleaching step is unacceptable, the stream can, however, be further purified by being treated with a membrane filtration process such as reverse osmosis. This technique provides a clean filtrate that can be recycled back to previous bleaching stages for further use. This has the benefit of reducing fresh water usage. Moreover, the concentrated chloride streams that result from the membrane filtration are relatively low in volume.

There may be some cases when extremely high pulp brightnesses are desired, for example, 92-95% GEB, where additional stages of bleaching may be required. An additional extraction and chlorine dioxide treatment would be a common choice, thereby creating a OₘZₘEDED bleach sequence.

Instead of using chlorine dioxide for fina brightening, the brightening bleaching may be conducted with hydrogen peroxide, as also shown in Fig. 1. This technique provides a completely chlorine-free bleaching cycle (such as an OₘZₘEP sequence), wherein no chlorinated materials are formed in the bleaching process and the liquid extraction product can be readily recycled without the necessity for cumbersome filtration techniques. When utilizing peroxides as the bleaching agent, however, the K No. of the pulp from either softwood or hardwood should be reduced to a level of about 6 prior to the ozonation step in order to obtain, as a final product following the peroxide bleaching stage, a pulp of acceptable brightness, i.e., a GE Brightness of greater than about 80%, since peroxide is not as effective at bleaching as is chlorine dioxide. Where a completely chlorine/chlorine dioxide-free process is desired, however, peroxide provides acceptable results.

Typical peroxide brightening agents and their use in this step are conventional, and one skilled in the art would know the appropriate concentration, types and use of such peroxide agents. Hydrogen peroxide is preferred.

The washed, further brightened pulp has a GE brightness of between about 70 and 95%, and preferably between about 80 and 95%. Also, the physical properties of this pulp are commensurate with those obtainable by pulp produced by conventional CEDED or OC/DED processes.

### 6. Washing Effluent Recycle

In any pulp process, filtrate management is an important factor in the overall economy or cost of operation of the process. The water which is used in the process requires both access to a suitable source and treatment of the effluent prior to discharge.

In an effort to reduce the water demand of the process, it is desirable to recycle as much of the effluent as possible. This practice cannot be used with processes utilizing chlorine or multiple steps of chlorine dioxide, since the effluents produced by these processes contain large amounts of chlorides produced by the by-products of such chemicals. Thus, recycling these effluents causes a build-up of chlorides which, in turn, causes either corrosion of processing equipment or the use of expensive materials of construction. In addition, such recycled effluents require substantial treatment before these effluents can be discharged from the mill, thus requiring further expenditures for equipment and treatment chemicals.

As illustrated in Fig. 4, use of either the conventional CEDED process or the OC/DED technique results in a significant disposal problem with regard to the effluents produced from the washing steps due to the high levels of chloride-containing compounds found therein. As noted above, these streams cannot be recycled, and are preferably treated before discharge into the environment. Recycling of effluent could be used to decrease the amount of water used, but then the process equipment may be subject to increased corrosion rates due to the increased chloride level in the recycled effluent.

In contrast, however, use of the OₘZₘED process of the invention results in formation of only a minimal amount of chlorinated material in the wash water, which water can be safely discharged, i.e., sewered, within most environmental protection standards. Alternately, this effluent may be treated by reverse osmosis to provide an even cleaner filtrate that may be recycled to previous bleaching stages as shown for further use without the build-up of chlorides. When a D bleaching stage is desired, steps may be taken to reduce the demand for chlorine dioxide. An Eₒ step may allow the pulp to achieve greater levels of brightness although additional expense is incurred by the use of additional sodium hydroxide and oxygen in this step. Also, there are known industry procedures for preparing chlorine dioxide whereby residual chlorine levels are minimized (e.g., the R8 process vs. the R3 process). These reduced chlorine level chemicals are preferred for use in the D stage to reduce the chloride levels of the wash water effluent.

Instead of OₘZₘED, one may use the OₘZₘEP process of the invention to obtain additional substantial advantages over the prior art in that no chlorinated compounds whatsoever are produced. This enables all of the effluent to be recycled without experiencing the problems of chloride build-up in the process wash water streams.

Accordingly, the process of the present invention achieves substantial advantages with respect to reductions in effluent volume, color, COD, BOD and chlorinated organics. Moreover, since the effluent used in the washing steps contains significantly reduced chloride levels compared to prior art processes which utilize chlorine, the washing unit vents will not be carrying chlorinated organic compounds or gases which require treatment prior to discharge.

### EXAMPLES

The scope of the invention is further described in connection with the following examples which are set forth for purposes of illustration only and which are not to be construed as limiting the scope of the invention in any manner. Unless otherwise indicated, all chemical percentages are calculated on the basis of the weight of oven dried (OD) fiber. Also, one skilled in the art would understand that the target brightness values do not need to be precisely achieved, as GEB values of plus or minus 2% from the target are acceptable. In all the examples having a D stage, except Example 11, an R-3 type of chlorine dioxide solution, known to contain a 6:1 ratio of dioxide to elemental chlorine, was used.

### EXAMPLE 1 (Comparative)

Loblolly pine chips were lab batch cooked according to the conditions in Table I to produce a conventional kraft pulp. The resulting pulp had a K No. of 22.6 and a viscosity of 27.1 cps. The kraft pulp was then subjected to conventional oxygen treatment (Tables II and V) followed by bleaching to a final target brightness of 83 GEB using both a conventional OC/DED sequence (Table III) and an OZₘED bleaching sequence (Tables IV and V). The ozone bleaching stage was run at 35% consistency with an ozone application of 0.61%.

As shown in Table VI and VII below, OZₘED bleaching under these conditions produced a pulp having acceptable strength properties compared to an 83% GE target brightness OC/DED baseline pulp. Under these conditions, the OZₘED pulp had marginal viscosity of 9.7 cps. The strength properties were measured on an OZₘED pulp where the final D-stage application was 2.5%. Target brightness was reached only with an excessive chlorine dioxide charge. The OZₘE pulps response to chlorine dioxide treatment shows that higher brightness can only be achieved by significantly increasing the ozone application, which then causes significant viscosity and strength loss of the pulp.

### EXAMPLE 2

A kraft/AQ brownstock was prepared in a laboratory batch digester from loblolly pine chips as described in Table VIII. The K No. of the resulting brownstock was 18.3 and the viscosity was 20.6 cps. The Kraft/AQ pulping conditions produced a pulp having a significantly lower lignin content than in Example 1 as evidenced by the K No., without unacceptable deterioration of pulp strength as evidenced by the viscosity.

The Kraft/AQ brownstock was then subjected to further bleaching using the conventional OC/DED sequence and the OZₘED sequence as shown in Tables II, III, IV and V to a target brightness of 83% GEB. Use of the Kraft AQ pulping technology achieved the goal of producing a starting pulp with a low K No., having acceptable viscosity properties, for the ozone bleaching sequence. The ozone bleaching stage was run at 35% consistency with an ozone application of 0.35% and 1.6% C10₂ was used in the final D stage to reach target brightness.

As shown in Tables IX and X below, the optical properties as measured by brightness response in the final chlorine dioxide stage were improved and strength properties were acceptable compared to the OC/DED baseline.

### EXAMPLE 3 (Comparative)

A pine Kraft brownstock having a K No. of about 24 was pressed to a consistency of about 30-36% by weight to produce a high consistency mat. The mat of brownstock was sprayed with a 10% sodium hydroxide solution in an amount sufficient to produce approximately 2.5 weight percent sodium hydroxide based on pulp dry weight. Dilution water was added in an amount sufficient to adjust the brownstock mat to about 27% consistency. The high consistency brownstock mat was then subjected to oxygen delignification using the following conditions: 110°C, 30 minutes, 551600 N/m² (80 psig) 0₂.

### EXAMPLE 4

Pine Kraft brownstock of Example 3 was introduced into a treatment vessel along with a sufficient volume of 10% NaOH solution to effect a 30% NaOH addition based on oven-dried pulp. Sufficient dilution water was added to obtain a brownstock consistency of about 3% by weight in the treatment vessel. The brownstock and the aqueous sodium hydroxide solution were uniformly mixed at room temperature by a ribbon mixer for about 15 minutes. The treated brownstock was then pressed to a consistency of about 27% by weight. After pressing, the sodium hydroxide on the fiber equaled about 2.5% as in Example 3. The treated brownstock was then delignified according to the oxygen delignification procedure described in Example 3. A comparison is shown in Table XI.

As can be seen from a comparison of Examples 3 and 4, a preferred method of the present invention of using a low consistency alkali addition followed by a high consistency oxygen treatment (Oₘ) produced a bleached brownstock having greater delignification (lower K No.) than the prior art methods, without any substantial change in strength properties.

As a result of the lower K No. pulp produced by this process, subsequent bleaching steps can be adjusted to accommodate the higher brightness, lower lignin containing pulp. Thus, the bleaching stages for such pulp require less bleaching agents or shorter bleaching times than for pulp which is not treated according to the present invention.

### EXAMPLE 5:

Pulp produced from pine in accordance with the Oₘ process of Example 4 of the present invention is compared to that produced conventionally (0) (i.e., with no low consistency alkaline treatment step). The average caustic dosage for high consistency oxygen delignification of brownstock pulp was found to be 22,5 kg (45 pounds) per oven dried tonne (ton) (1b/t) or 2.3%. At that level, the average reduction in K No. across the oxygen delignification reactor was 10 units. For the same level of caustic applied to pulp according to a preferred treatment step, an average K No. drop during delignification was found to be 13 units: a 30% improvement compared to the conventional process.

This advantage in delignification selectivity can also be shown by a comparision of pulp viscosity. The average K No. and viscosity for conventional pulp was 12.1 and 14.4 cps, respectively. For the preferred treatment process of the invention, the average K No. at essentially the same viscosity (14.0 cps) was 8.3.

Delignification selectivity can also be expressed as the change in viscosity versus the change in K No. between brownstock and the corresponding treated pulps. Oxygen delignification selectivity decreases rather rapidly when the change in K No. begins to exceed 10 K No. units. The decrease in selectivity is observed as a rapid increase in the change in viscosity for a given change in K No. As an example, for a change in K No. of 12 units, the corresponding change in viscosity is expected to be 12 to 13 cps. By contrast, for the same change in K No. (12) obtained by delignified pulps which have been treated using the preferred method, the change in viscosity was found to be about 6 cps. The change in viscosity per change in K No. appears to be constant up to a 16 to 17 K No. unit change for pulps obtained using the preferred treatment process of the invention. The results are shown in Table XII.

### EXAMPLE 6

A southern pine pulp was produced in an operating 600 TPD fine paper mill using the modified oxygen delignification process (0ₘ) having the conditions of Table II in combination with the uniform alkali treatment as described in Examples 4 and 5 and the conditions as shown in Table XIII below. The O-stage pulp produced by this novel method had the properties needed to successfully complete the bleaching process using ozone, as described in the embodiment of this invention. The oxygen stage pulp had a K No. of 7.9 (compared to a typical conventional O-stage K No. of about 12). Viscosity of the delignified pulp was 15 cps and was not significantly reduced by the high degree of delignification obtained by the use of the modified oxygen process. This pulp could then be further bleached with ozone, utilizing any of the numerous process embodiments described herein to produce a pulp having acceptable final strength and optical properties.

C/DED bleaching of this pulp was completed in the laboratory, as described in Table XIV, to provide a baseline for comparison of properties.

The ozone bleaching stage was carried out in a pilot plant reactor as shown in Fig. 2. Conditions of operation of the pilot plant reactor are shown in Table XV.

The ozone bleached pulp generated in the pilot plant reactor was then treated in extraction and chlorine dioxide stages in the laboratory, as described in Table V above, to produce a final bleached pulp product at target brightness. A final D stage charge of only 1.0 % C10₂ was used on the fiber.

The strength and optical properties of the ozone bleached pulp were acceptable compared to the conventional OC/DED baseline and the results of the comparison are shown in Tables XVI and XVII below.

### EXAMPLE 7

To further exemplify the utility and range of applicability of the process of this invention, a southern hardwood fiber, from mixed hardwood comprising predominantly gum and oak, was bleached with ozone in the pilot plant described in Example 6 above. A conventional oxygen stage pulp produced in the 600 TPD mill was treated with ozone in the pilot plant reactor. The oxygen stage pulp had a K No. of 5.7 and a viscosity of 14.1.

A portion of the O stage pulp was final bleached by the conventional C/DED sequence in the laboratory to provide a baseline for comparison. The C/DED conditions are shown in Table XVIII.

The ozone reactor treatment conditions are shown in Table XIX. The pilot plant Zₘ stage pulp was then final bleached by conventional E and D stages as shown in Table XX to a target brightness. A D-stage C10₂ charge of only 0.35% was used on OD fiber. Strength and brightness properties were acceptable compared to the baseline as shown in Tables XXI and XXII.

### EXAMPLE 8:

Comparison tests similar to Example 5 were carried out for laboratory produced Kraft hardwood pulp, from mixed hardwood comprising predominantly gum and oak. Again, it was found that a significantly larger K No. drop across the oxygen delignification reactor using the modified oxygen process (Oₘ) is achieved compared to conventional oxygen processing (O). The average caustic dosage for hardwood was 13.5 kg/tonne (27 lb/t), or 1.4%. This produced a K No. drop of about 5 units during the oxygen step. For the same level of caustic utilized according to the modified oxygen process of the present invention, an average K No. drop of about 7.3 units was obtained, an increase of almost 50%.

This advantage in delignification selectivity can also be shown by comparing pulp viscosity. The average hardwood K No. and viscosity were found to be 7.6 and 16 cps, respectively. For the invention, a K No. of 6 and a viscosity of 17.7 was obtained. Also, the K No. at the same viscosity as the non-treated pulp (16 cps), was found to be 5.8.

Delignification selectivity can also be expressed in terms of the change in viscosity versus the change in K No. between brownstock and the corresponding modified oxygen treated pulps. In comparing pulps which are conventionally oxygen treated with those of the invention, there is a greater decrease in delignification selectivity for increased degrees of delignification. For a change in K No. of 4 units, the average change in viscosity was 4 cps for pulps produced by the conventional process. By contrast, the change in K No. for the same change in viscosity for pulps produced by the modified oxygen method was 7 units. Expressed in terms of a delignification selectivity ratio, the selectivity for the modified method was 1.8 K No./cps and that for the conventional process was 1 K No./cps, an increase of 80%. Results are shown in Table XXIII.

### EXAMPLE 9

A series of experiments were carried out in the pilot plant reactor using pulp from a 600 TPD fine paper mill with a conventional oxygen delignification stage (O). These experiments were performed to illustrate the effect of pH on the ozone bleaching process using southern hardwoods. Reactor operating conditions were held constant at the conditions shown in Table XXIV with the pH of the ozone stage being the only variable.

As can be seen from Table XXV below, the effect of pH on the ozone bleaching process is significant with lower pH beneficially improving the selectivity of the bleaching process.

### EXAMPLE 10

A number of comparative properties are of interest to illustrate the beneficial effects of producing fully bleached pulps using the OZₘED process. Typical operating data and effluent measurements were collected from operating mills using the CEDED and OC/DED bleaching sequences on Southern pine. These properties were compared to those of effluents produced by the OZₘED sequence, using the OZₘED pulp and effluent prepared in Example 1. For the conventional CEDED sequence see Table XXVI, for the conventional OC/DED sequence see Tables II and III above and for the 0ZₘED sequence see Tables IV and V above. It should be noted that the CEDED sequence effluent is the combined C, E₁, D₁, E₂ and D₂ effluent. The OC/DED effluent is the C/D, E and D combined effluent and the OZₘED effluent is the D stage effluent, each representing the several effluent properties. As shown in Table XXVII below, the ozone bleaching sequence substantially reduces the environmental impact of the effluent from the bleaching process. To determine color, EPA method 110.2 was used. From this data, it can be seen that the present invention provides a discharge effluent having a color of no greater than about 1 kg/tonne (2 pounds per ton), a BOD₅ value of no greater than about 1 kg/tonne (2 pounds per ton) and an amount of total organic chloride of no greater than about 1 (2) and preferably less than about 0.4 (0.8).

### EXAMPLE 11

Southern pine kraft pulp was bleached using three modifications of the basic OZED sequence. In the first sequence (OZₘED), the pulp was bleached as in Tables IV and V with conventional oxygen, modified ozone, caustic extraction and chloride dioxide as produced in the R-3 sequence with a Cl0₂/Cl₂ ratio of 6:1. In the second sequence, the modified oxygen process (Oₘ) was utilized and again the final stage used an R-3 type of chlorine dioxide. In the third sequence, the modified oxygen process (Oₘ) was used once again, and an R-8 chlorine dioxide solution was employed with 95:1 ratio in the final stage. Table XXVIII demonstrates the positive environmental impact offered with the use of the modified oxygen process (Oₘ). The R-8 bleach liquor also had a positive effect.

### EXAMPLE 12

Southern loblolly pine pulps were prepared by the kraft and kraft/AQ pulping processes as described in Tables I and VIII above. These pulps were further subjected to conventional and modified oxygen delignification as described in Examples 4 and 5 to show the effect of combining these processes (for extending delignification with minimal impact on pulp strength) on the ozone bleaching sequence. As can readily be seen from Table XXIX, these processes produce an additive effect. Extremely low 0ₘZₘE K Nos. can be reached with little impact on final viscosity. Conversely, the amount of ozone needed to reach a target 0ₘZₘE K No. of about 3.5 for the previously described ozone bleaching process can be substantially reduced. In addition, the additive effect produces a southern pine pulp that can be fully bleached by an 0ₘZₘEP process where a very low 0ₘZₘE K No. is required for a functional peroxide stage.

### Example 13

Southern softwood, i.e., loblolly pine, was bleached to target brightness of 83 GEB using the conventional CEDED sequence as shown in Table XXVI, using the conventional OC/DED sequence as shown in Tables II and III above and using the OZₘED sequence as shown in Tables IV and V above. Wood based dirt was refined and added to the OZₘED starting brownstock at a level of 0.75% by weight to examine the ability of this sequence to remove dirt compared to CEDED and OC/DED bleaching. Dirt properties of the three sequences, measured as Effective Black Area, bark and shives, were equivalent.

### Example 14

This example illustrates the range of applicability of the ozone bleaching process of the invention. Bleached pulps can be produced over a wide range of product brightnesses, utilizing appropriate combinations of ozone and chlorine dioxide charges to minimize environmental impacts and operating costs. As shown in Table XXX below, products having brightness from above 65% GEB can be produced by various combinations of ozone and chlorine dioxide while retaining reasonable strength properties.

## Claims

1. A process for the manufacture of a substantially uniformly bleached pulp from a lignocellulosic material which comprises preparing an intermediate pulp with a reduced lignin portion by chemically digesting (4) the lignocellulosic material followed by oxygen delignifying (26) the pulp thereby obtained which process is further characterized in that:
a) the pH of the intermediate pulp is adjusted (42) to the range of about 1 to 4.
b) the consistency of the intermediate pulp is adjusted (48) to a high consistency of about 20% to 50%.
c) the intermediate pulp is comminuted (56) into discrete particle, the majority of which have a size of less than about 5mm.
d) the intermediate pulp obtained after a), b), c), is subjected to a delignifying treatment by turbulently mixing it with an ozone containing gaseous mixture in a dynamic reaction zone (58) for a sufficient time and at a temperature sufficient to allow access of the ozone to substanially all of the intermediate pulp for reaction therewith while the said pulp is conveyed (62) through substantially all of the reaction zone, thus obtaining a further substantially uniform delignification of a significant portion of the pulp.

2. The process of claim 1 which comprises chemically digesting the lignocellulosic material by Kraft pulping, Kraft AQ pulping or extended delignification.

3. The process according to claim 1 or 2, wherein the oxygen delignification step comprises forming a low to medium consistency pulp; treating the low to medium consistency pulp with an aqueous solution of an alkaline material for a predetermined time and at a predeterined temperature relative to the quantity of the alkaline material to substantially uniformly distribute the alkaline material throughout the low to medium consistency pulp; raising the consistency of the pulp to a high consistency of about 20% to 50% and subjecting the resulting high consistency pulp to high consistency oxygen delignification to obtain the intermediate pulp.

4. The process of claim 1, 2, or 3, wherein the final GE brightness of the bleached pulp is at least about 50%, the viscosity thereof is greater than about 10 cps, and wherein the amount of lignin is indicated by an intermediate pulp K No. of about 10 or less and the viscosity of the intermediate pulp is greater than about 13 cps.

5. The process of claim 1, 2, 3 or 4, wherein the lignocellulosic material is softwood, the final brightness of the bleached pulp is at least about 50%, the viscosity thereof is greater than about 10 cps, and wherein the amount of lignin is indicated by an intermediate pulp K No. of about 7-10 and the viscosity of the intermediate pulp is greater than about 13 cps.

6. The process of claim 1, 2, 3, 4 or 5, wherein the lignocellulosic material is a hardwoord, the final GE brightness of the bleached pulp is at least about 55%, the viscosity thereof is greater than about 10 cps, and wherein the amount of lignin is indicated by an intermediate pulp K No. of about 5-8 and the viscosity of the intermediate pulp is greater than about 13 cps.

7. The process of claim 4, 5 or 6 wherein the amount of lignin contained in the pulp after ozone delignification is indicated by a bleached pulp K No. of about 3 to 4.

8. The process of claim 1 which further comprises bleaching the pulp after ozone delignification with a brightening agent to increase the GE brightness of the bleached pulp.

9. The process of claim 8 which further comprises combining the bleached pulp with an effective amount of alkaline material in an alkaline aqueous solution at a predetermined temperature, correlated to the amount of alkaline material combined, to solubilize a substantial portion of any lignin remaining in the bleached pulp; and thereafter extracting a portion of the aqueous alkaline solution so as to remove substantially all of the solubilized lignin therefrom and form an extracted pulp prior to bleaching with the brightening agent.

10. The method of claim 8 wherein the brightening agent is chlorine dioxide or a peroxide.

11. The process of claim 1 wherein:
the lignocellulosic material is chemically digested to form a pulp having first K No. and first viscosity values;
said pulp is delignified with oxygen to form a partially delignified pulp having a second K No. lower than said first K No., and which is sufficient to enable the partially delignified pulp to be further delignified with ozone while maintaining viscosity at a level such that cellulose components of said partially delignified pulp have not been significantly chemically degraded by the oxygen delignification; and
the partially delignified pulp is further delignified by the ozone to obtain a substantially delignified pulp having a third K No. which is significantly reduced below said second K No. of said partially delignified pulp and having a GE brightness value substantially above that of the partially delignified pulp while maintaining viscosity and without aggressively chemically attacking cellulose components of the pulp to avoid substantially reducing the strength of the pulp.

12. The process of claim 11 wherein the partially delignified pulp contains an amount of lignin which, after ozone delignification, permits the pulp to attain the certain GE brightness, and also has a viscosity which is sufficiently high to compensate for viscosity decreases during ozone delignification, thus permitting the substantially delignified pulp to attain the certain strength.

13. The process of claim 11 which further comprises combining the substantially delignified pulp with an effective amount of alkaline material in an alkaline aqueous solution at a predetermined temperature, correlated to the amount of alkaline material combined, to solubilize a substantial portion of any lignin remaining in the substantially delignified pulp; and thereafter extracting a portion of the aqueous alkaline solution so as to remove substantially all of the solubilized lignin therefrom and form a substantially lignin-free pulp.

14. The process of claim 13 which further comprises bleaching the substantially lignin-free pulp to a brightness value which is substantially higher than that of the substantially delignified pulp.

15. The process of claim 11 wherein the viscosity of said partially delignified pulp is maintained at greater than about 13 cps.

16. The process of claim 15 wherein said partially delignified pulp is maintained at a viscosity decrease of about 30% or less of said first value.

17. The process of claim 11 wherein said lignocellulosic material is a hardwood.

18. The process of claim 17 wherein said first K No. is between about 10-14.

19. The process of claim 17 wherein said first viscosity value is between about 21-28 cps.

20. The process of claim 17 wherein said second K No. is between about 5-8.

21. The process of claim 20 wherein said third K No. is less than about 5.

22. The process of claim 11 wherein said lignocellulosic material is a softwood.

23. The process of claim 22 wherein said first K No. is between about 20-24.

24. The process of claim 22 wherein said second K No. is between about 7-10.

25. The process of claim 11 wherein the oxygen delignification treatment is carried out on pulp of medium consistency.

26. The process of claim 11 wherein the partial delignification step further comprises:
treating said pulp with a quantity of alkaline material in an aqueous alkaline solution for a predetermined time and at a predetermined temperature correlated to the quantity of alkaline material to substantially complete a substantially uniform distribution of the alkaline material throughout the pulp;
increasing the consistency of the pulp after the completion of the treating step; and
subjecting the increased consistency alkaline material containing pulp to high consistency oxygen delignification to obtain a partially delignified pulp.

27. The process of claim 11 wherein the viscosity of said substantially delignified pulp is maintained at greater than about 10 cps.

28. The process of claim 27 wherein said substantially delignified pulp is maintained at a viscosity decrease of about 30% or less of the viscosity of said partially delignified pulp.

29. The process of claim 11 wherein the further delignifying step additionally comprises:
increasing the consistency of said partially delignified pulp;
comminuting said increased consistency pulp to a predetermined particle size; and
uniformly contacting said comminuted pulp with said effective amount of ozone as the pulp is advanced through the process.

30. The process of claim 29 wherein the particle size of said increased consistency pulp is comminuted to one that facilitates uniform contact with ozone without causing significant degradation of the cellulose components of the pulp.

31. The process of claim 30 wherein the pulp is comminuted to about 5 mm and advanced through the process in a manner to avoid a non-uniform application of the ozone to the pulp.

32. The process of claim 31 wherein the comminuted pulp is advanced cocurrently with the ozone.

33. The process of claim 31 wherein the comminuted pulp is advanced countercurrently to the ozone.

34. The process of claim 14 wherein the substantially lignin free pulp is bleached with chlorine dioxide.

35. The process of claim 14 wherein the substantially lignin free pulp is bleached with a peroxide.

36. The process of claim 34 or 35 wherein the bleaching step raises the GE brightness of said substantially lignin free pulp to at least about 70%.

37. The process of claim 34 or 35 wherein the bleaching step raises the GE brightness of said substantially lignin free pulp to at least about 80%.

38. The process of claim 34 or 35 wherein the bleaching step raises the GE brightness of said substantially lignin free pulp to at least about 90%.

39. The process of claim 1 wherein the oxygen delignified pulp has a K No. of about 10 or less and a viscosity of greater than about 13 cps after oxygen delignification; and the ozone delignified pulp has a K No. of about 5 or less, a viscosity of greater than about 10 and a GE brightness of at least about 50% after ozone delignification.

40. The process of claim 39 wherein the lignocellulosic material is a softwood and is partially delignified to a pulp having a K No. of about 7 to 10 and a viscosity of above about 13 before further delignification with ozone.

41. The process of claim 40 wherein the softwood pulp has a K No. of about 3 to 4, a viscosity of above about 10 and a GE brightness of at least about 50% after said further delignification with ozone.

42. The process of claim 39 wherein the lignocellulosic material is a hardwood and is partially delignified to a pulp having a K No. of about 5 to 8 and a viscosity of above about 13 before further delignification with ozone.

43. The process of claim 42 wherein the hardwood pulp has a K No. of about 3 to 4, a viscosity of above about 10, and a GE brightness of at least about 55% after further delignification with ozone.

44. The process of claim 39 which further comprises: combining the substantially delignified pulp with an effective amount of alkaline material in an aqueous alkaline solution for a predetermined time and at a predetermined temperature correlated to the quantity of alkaline material to solubilize a substantial portion of any lignin which remains in the pulp, and
thereafter extracting a portion of the aqueous alkaline solution so as to remove substantially all of the solubilized lignin therefrom and form a substantially lignin-free pulp.

45. The process of claim 44 wherein said extracting step raises the brightness of the pulp by about 2%.

46. The process of claim 44 which further comprises bleaching the substantially lignin-free pulp with one of chlorine dioxide or a peroxide to raise the GE brightness to at least about 70%.

47. The process of claim 46 wherein the GE brightness is raised to at least about 80%.

48. The process of claim 46 wherein the GE brightness is raised to at least about 90%.

49. The process of claim 44 wherein the lignocellulosic material is partially delignified by an oxygen delignification treatment.

50. The process of claim 50 wherein the oxygen delignification treatment is carried out on pulp of medium consistency.

51. The process of claim 44 wherein the lignocellulosic material is partially delignified by:
forming a pulp having a relatively low consistency of less than 10% by weight;
treating the low consistency pulp with a quantity of alkaline material in an aqueous alkaline solution for a predetermined time and at a predetermined temperature correlated to the quantity of alkaline material to substantially complete a substantially uniform distribution of the alkaline material throughout the pulp;
increasing the consistency of the pulp to at least about 20% by weight after completion of the treating step; and
subjecting the increased consistency alkaline material containing pulp to high consistency oxygen delignification to obtain a partially delignified pulp having a K No. of about 9 or less and a viscosity of about 13 or higher.

52. The process of claim 1 wherein:
the oxygen delignifying step comprises:
reducing the consistency of the pulp to a consistency of less than 10% by weight;
treating the reduced consistency pulp with a quantity of alkaline material in a aqueous alkaline solution for a predetermined time and at a predetermined temperature correlated to the quantity of alkaline material to substantially complete a substantially uniform distribution of the alkaline material throughout the pulp;
increasing the consistency of the pulp to at least about 20% by weight after completion of the treating step; and
subjecting the increased consistency alkaline material containing pulp to high consistency oxygen delignification to obtain a partially delignified pulp having a K No. of about 9 or less and a viscosity of greater than about 13 cps;
the oxygen delignifying step obtains a substantially delignified pulp having a K No. of about 5 or less, a viscosity of greater than about 10 and a GE brightness of at least about 50%;
and the process further comprises:
combining the ozone delignified pulp with an effective amount of alkaline material in an aqueous alkaline solution for a predetermined time and at a predetermined temperature correlated to the quantity of alkaline material to solubilize a substantial portion of any lignin which remains in the pulp;
extracting a portion of aqueous alkaline solution so as to remove substantially all of the solubilized lignin therefrom and form a substantially lignin-free pulp; and
bleaching the substantially lignin-free pulp to raise the GE brightness thereof to at least about 70%.

53. The process of claim 52 wherein the GE brightness is raised to at least about 80%.

54. The process of claim 52 wherein the GE brightness is raised to at least about 90%.

55. The process of claim 52 wherein the lignocellulosic material is a softwood and is partially delignified to a K No. of about 8 to 9 and a viscosity of greater than about 14 before further delignification with ozone.

56. The process of claim 55 wherein the softwood pulp has a K No. of between about 3 to 4, a viscosity of above about 10, and a GE brightness of at least about 54% after said further delignification with ozone.

57. The process of claim 52 wherein the lignocellulosic material is a hardwood and is partially delignified to a K No. of about 6 to 7 and a viscosity of above about 15 before said further delignification with ozone.

58. The process of claim 57 wherein the hardwood pulp has a K No. of between about 3 to 4, a viscosity of above about 10, and a GE brightness of at least about 63% after said further delignification with ozone.

59. The process of claim 52 wherein the partially delignified lignocellulosic material is obtained by Kraft pulping, Kraft-AQ pulping or extended delignification of a lignocellulosic material.

60. The process of claim 52 which comprises decreasing the K No. of the increased consistency pulp by at least about 60% during the oxygen delignification step without significantly damaging the cellulose components of the pulp.

61. The process of claim 52 wherein the pulp is subjected to the high consistency oxygen delignification without substantially changing the viscosity of the pulp.

62. The process of claim 52 which comprises decreasing the ratio of K No. to viscosity of the pulp during the oxygen delignification step by at least 25%.

63. The process of claim 52 wherein the consistency of the pulp which is treated with the aqueous alkaline solution prior to oxygen delignification ranges between about 1 and 4.5% by weight.

64. The process of claim 52 wherein the consistency of the pulp is increased to between about 25 and 35% by weight prior to the oxygen delignification step.

65. The process of claim 52 wherein the amount of alkaline material distributed throughout the low consistency pulp prior to oxygen delignification ranges from about 15 to 30% by weight based on the dry weight of the pulp.

66. The process of claim 65 wherein the aqueous alkaline solution has a concentration of alkaline material of between about 20 and 120 g/l, so that the concentration of alkaline material in the low consistency pulp ranges from about 6.5 to 13 g/l.

67. The process of claim 52 wherein the alkaline treating step is conducted for a time of between about 1 and 15 minutes at a temperature of between about 90 and 150°F.

68. The process of claim 52 wherein the initially formed pulp is brownstock pulp and further wherein at least a portion of the liquid obtained from the alkaline solution during the pulp consistency increasing step is recycled to the alkaline treating step.

69. The process of claim 1 wherein:
the pulp is initially formed as a brownstock pulp having a K No. of from about 10-24 by Kraft pulping, Kraft-AQ pulping or extended delignification of the lignocellulosic material;
the oxygen delignifying step comprises:
decreasing the consistency of said pulp to about 1 to 4.5% by weight;
treating the decreased consistency pulp with a quantity of alkaline material in an aqueous alkaline solution having a concentration of alkaline material of between about 20 and 120 g/l for a time of between about 1 and 15 minutes and at a temperature of between about 90 and 150°F such that the concentration of alkaline material in the decreased consistency pulp during this treating step ranges from about 6.5 to 13 g/l, so as to substantially complete a substantially uniform distribution of the alkaline material throughout the pulp;
increasing the consistency of the alkaline treated pulp to between about 25 to 35% by weight; and
subjecting the increased consistency pulp to high consistency oxygen delignification without substantially changing the viscosity of the pulp to form a partially delignified pulp having a K No. of about 10 or less and a viscosity of greater than about 13, wherein the ratio of K No. to viscosity of said pulp is decreased by at least abcut 25% during oxygen delignification;
the ozone delignifying step obtains a substantially delignified pulp having a K No. of about 5 or less, a viscosity of greater than about 10 and a GE brightness of at least about 50%;
and the process further comprises:
combining the substantially delignified pulp with an effective amount of alkaline material in an aqueous alkaline solution for a predetermined time and at a predetermined temperature correlated to the quantity of alkaline material to solubilize a substantial portion of any lignin which remains in the pulp;
extracting a portion of aqueous alkaline solution so as to remove substantially all of the solubilized lignin therefrom and form a substantially lignin-free pulp; and
bleaching the substantially lignin-free pulp to raise the GE brightness thereof to at least about 70%.

70. The process of claim 69 wherein the GE brightness is raised to at least about 80%.

71. The process of claim 69 wherein the GE brightness is raised to at least about 90%.

72. The process of claim 69 which comprises decreasing the K No. of the increased consistency pulp by at least about 60% during the oxygen delignification step without significantly damaging the cellulose components of the pulp.

73. The process of claim 69 wherein the substantially lignin-free pulp is bleached with chlorine dioxide or a peroxide.

74. The process of claim 73 wherein the peroxide is hydrogen peroxide.

75. The process of claim 69 which further comprises adding a chelating agent to said pulp prior to ozone delignification to render metal ions substantially non-reactive to ozone.

76. The process of claim 75 wherein the chelating agent is DTPA, EDTA or oxalic acid.

77. The process of claim 69 which further comprises adjusting the pH of the pulp to a range of about 1 to 4 by adding to the pulp a sufficient quantity of an acidic material prior to ozone delignification.

78. The process of claim 69 which further comprises increasing the consistency of the pulp to between about 25-50% by weight prior to ozone delignification.

79. The process of claim 78 wherein the consistency of the pulp is increased to between about 35-45% by weight prior to ozone delignification.

80. The process of claim 69 which comprises comminuting said pulp to a diameter of less than about 5 mm after oxygen delignification and prior to ozone delignification.

81. The process of claim 69 which further comprises maintaining the pulp at a temperature of less than about 120°F during ozone delignification.

82. The process of claim 69 wherein the ozone is provided by a mixture comprising ozone and oxygen.

83. The process of claim 82 wherein the ozone concentration in the mixture is between about 1 and 8 percent by volume.

84. The process of claim 69 wherein the ozone is provided by a mixture of ozone and air.

85. The process of claim 84 wherein the ozone concentration is between about 1 and 4 percent by volume.

86. The process of claim 69 which comprises advancing the partially delignified pulp during the ozone delignification step in a manner which subjects substantially all the pulp to ozone.

87. The process of claim 86 which comprises introducing the ozone countercurrently to the advancing pulp.

88. The process of claim 86 which comprises introducing the ozone cocurrently with the advancing pulp.

89. The process of claim 1 wherein:
the oxygen delignified pulp has a K No. of about 10 or less and a viscosity of greater than about 13 cps;
the ozone delignifying step comprises:
adding a chelating agent to said pulp to render metal ions therein substantially non-reactive to ozone;
adjusting the pH of said pulp to a range of about 1 and 4 by adding a sufficient quantity of an acidic material thereto;
increasing the consistency of said pulp to between about 25 and 50%;
comminuting said increased consistency pulp to a diameter of less than about 5 mm; and
delignifying said increased consistency pulp with an effective amount of ozone for a sufficient time by advancing the comminuted pulp in a manner which subjects substantially all the pulp to the ozone to obtain a substantially delignified pulp having a K No. of about 5 or less, a viscosity of greater than about 10 and a GE brightness of at least about 50%;
and the process further comprises:
combining the substantially delignified pulp with an effective amount of alkaline material in an aqueous alkaline solution for a predetermined time and at a predetermined temperature correlated to the quantity of alkaline material to solubilize a substantial portion of any lignin which remains in the pulp;
extracting a portion of aqueous alkaline solution so as to remove substantially all of the solubilized lignin therefrom and form a substantially lignin-free pulp; and
bleaching the substantially lignin-free pulp with chlorine dioxide to raise the GE brightness thereof to at least about 70%.

90. The process of claim 89 wherein the GE brightness is raised to at least about 80%.

91. The process of claim 89 wherein the GE brightness is raised to at least about 90%.

92. The process of claim 89 wherein the pulping step comprises Kraft pulping and the oxygen delignification step decreases the K No. of the pulp by at least about 60% without significantly damaging the cellulose components of the pulp or without substantially changing the viscosity of the pulp.

93. The process of claim 92 wherein the pulping step comprises Kraft AQ pulping.

94. The process of claim 93 wherein the oxygen delignification step decreases the K No. of the pulp by at least about 60% without significantly damaging the cellulose components of the pulp or without substantially changing the viscosity of the pulp.

95. The process of claim 89 wherein the pulping step comprises the combination of Kraft AQ pulping and extended delignification, and the oxygen delignification step decreases the K No. of the pulp by at least about 60% without significantly damaging the cellulose components of the pulp or without substantially changing the viscosity of the pulp.

96. The process of claim 89 wherein during ozone delignification the pulp is advanced in a manner so that the pulp is maintained at a temperature of less than about 120°F.

97. The process of claim 89 wherein the chelating agent and acid are added to said pulp in a mixing chest.

98. The process of claim 97 wherein at least a portion of the liquid separated from the pulp during the consistency increasing step is recycled to the mixing chest.

99. The process of claim 97 wherein the pulp is advanced cocurrently with the ozone.

100. The process of claim 97 wherein the pulp is advanced countercurrently with the ozone.

101. The process of claim 1 wherein:
the oxygen delignified pulp has a K No. of about 10 or less and a viscosity of greater than about 13 cps;
the ozone delignifying step comprises:
adding a chelating agent to said pulp to render metal ions therein substantially non-reactive to ozone;
adjusting the pH of said pulp to a range of about 1 and 4 by adding a sufficient quantity of an acidic material thereto;
increasing the consistency of said pulp to between about 25 and 50%;
comminuting said increased consistency pulp to a diameter of less than about 5 mm; and
delignifying said increased consistency pulp with an effective amount of ozone for a sufficient time to obtain a substantially delignified pulp having a K No. of about 5 or less, a viscosity of greater than about 10 and a GE brightness of at least about 50%;
and the process further comprises:
combining the substantially delignified pulp with an effective amount of alkaline material in an aqueous alkaline solution for a predetermined time and at a predetermined temperature correlated to the quantity of alkaline material to solubilize a substantial portion of any lignin which remains in the pulp;
extracting a portion of aqueous alkaline solution so as to remove substantially all of the solubilized lignin therefrom and form a substantially lignin-free pulp; and
bleaching the substantially lignin-free pulp with a peroxide to raise the GE brightness thereof to at least about 70%.

102. The process of claim 101 wherein the GE brightness is raised to at least about 80%.

103. The process of claim 101 wherein the GE brightness is raised to at least about 90%.

104. The process of claim 101 wherein the pulping step comprises Kraft pulping and the oxygen delignification step decreases the K No. of the pulp by at least about 60% without significantly damaging the cellulose components of the pulp or without substantially changing the viscosity of the pulp.

105. The process of claim 101 wherein the pulping step comprises Kraft AQ pulping.

106. The process of claim 105 wherein the oxygen delignification step decreases the K No. of the pulp by at least about 60% without significantly damaging the cellulose components of the pulp or without substantially changing the viscosity of the pulp.

107. The process of claim 101 wherein the pulping step comprises the combination of Kraft AQ pulping and extended delignification, and the oxygen delignification step decreases the K No. of the pulp by at least about 60% without significantly damaging the cellulose components of the pulp or without substantially changing the viscosity of the pulp.

108. The process of claim 89 or 101 wherein the ozone delignification reduces the K No. of the pulp by at least 50%.

109. The process of claim 89 or 101 wherein the bleaching step raises the GE brightness of the pulp by at least 50%.

110. The process of claim 109 wherein the GE brightness of the pulp is increased to at least 83%.

111. The process of claim 1 wherein:
the pulp is washed between the chemical digesting and oxygen delignifying steps, with said pulp after the oxygen delignification step having a K No. of about 10 or less and a viscosity of greater than about 13 cps;
and the process further comprises:
washing the oxygen delignified pulp;
conducting the ozone delignification step to obtain a substantially delignified pulp having a K No. of about 5 or less, a viscosity of greater than about 10 and a GE brightness of at least about 50%;
washing the substantially delignified pulp;
combining the substantially delignified pulp with an effective amount of alkaline material in an aqueous alkaline solution for a predetermined time and at a predetermined temperature correlated to the quantity of alkaline material to solubilize a substantial portion of any lignin which remains in the pulp;
extracting a portion of the aqueous alkaline solution so as to remove substantially all of the solubilized lignin therefrom and form substantially lignin-free pulp;
washing the substantially lignin-free pulp;
bleaching the substantially lignin-free pulp with one of chlorine dioxide or a peroxide to raise the GE brightness thereof to at least about 70%; and
washing the bleached pulp.

112. The process of claim 111 wherein the GE brightness is raised to at least about 80%.

113. The process of claim 111 wherein the GE brightness is raised to at least about 90%.

114. The process of claim 111 wherein the bleached pulp washing step comprises washing said pulp with fresh water, and separating the pulp from the resulting wash water effluent.

115. The process of claim 111 wherein the bleaching step utilizes chlorine dioxide and the bleached pulp wash water effluent is discharged.

116. The process of claim 111 wherein the bleaching step utilizes chlorine dioxide and the bleached pulp wash water effluent is treated by reverse osmosis to form a treated filtrate and at least a portion of said treated filtrate is then directed to the substantially lignin-free pulp washing step.

117. The process of claim 111 wherein the bleaching step utilizes a peroxide and at least a portion of the bleached pulp is recycled to the step wherein the substantially lignin-free pulp is washed.

118. The process of claim 116 or 117 wherein the substantially lignin-free pulp washing step comprises washing said pulp with bleached pulp wash water, separating the pulp from the resulting wash water and directing at least a portion of said wash water to the substantially delignified pulp washing step.

119. The process of claim 118 wherein the substantially delignified pulp washing step comprises washing said pulp with the substantially lignin-free pulp wash water, separating the pulp from the resulting wash water and directing at least a portion of said wash water to the partially delignified pulp washing step.

120. The process of claim 119 wherein the partially delignified pulp washing step comprises washing said pulp with substantially delignified pulp wash water, separating the pulp from the resulting wash water and directing at least a portion of said wash water to the pulp washing step.

121. The process of claim 120 wherein the pulp washing step comprises washing said pulp with partially delignified pulp wash water, separating the pulp from the resulting wash water, and collecting and concentrating said wash water prior to incineration in a recovery boiler.

122. The process of claim 111 or 121 wherein the bleaching step utilizes chlorine dioxide having a minimum chlorine content.

123. The process of claim 111 or 121 wherein the water demand for the washing steps is substantially reduced compared to conventional CEDED or OC/DED processes.

124. The process of claim 115 wherein the discharge effluent has a color of no greater than about 2 pounds per ton, a BOD₅ value of no greater than about 2 pounds per ton and an amount of total organic chlorides of no greater than about 2.

125. The process of claim 75 wherein the chelating agent is a polycarboxylate or polycarboxylate derivative.

126. The process of claim 75 wherein the chelating agent is used in an amount of 0.1 to 0.2% by weight of oven dry pulp.

127. The process of claim 75 wherein the pulp is acidified to a pH from about 1 to about 4 prior to the chelating agent treatment step.

128. The process of claim 75 wherein the pulp, after ozone bleaching, is brightened with a peroxide.

## Patentansprüche

1. Verfahren für die Bereitung eines nahezu einheitlich gebleichten Breis aus Lignin-Zellstoff-Material, welches Verfahren die Bereitung eines Übergangsbreis mit reduziertem Lignin-Gehalt durch chemisches Erschließen (4) des Lignin-Zellstoff-Materials mit anschließender Sauerstofferschließung (26) des dabei erhaltenen Breis umfaßt, welches Verfahren durch die nachfolgenden Schritte gekennzeichnet ist:
a) der pH-Wert des Übergangsbreis wird im Bereich von etwa 1 bis 4 eingestellt (42);
b) die Konsistenz des Übergangsbreis wird auf einen hohen Wert von etwa 20% bis 50% eingestellt;
c) der Übergangsbrei wird zu diskreten Teilchen zerkleinert (56), deren größter Teil eine Dimension von weniger als etwa 5 mm hat;
d) der Übergangsbrei, der nach den Schritten a), b), c) erhalten worden ist, wird einer Lignin-Extraktion unterworfen, indem er im Wirbelverfahren mit einer ozonhaltigen Gasatmosphäre in einer dynamischen Reaktionszone (58) vermischt wird, und zwar während einer Dauer und bei einer Temperatur, die dazu ausreichen, daß das Ozon nahezu den ganzen Übergangsbrei durchdringen kann, um damit eine Reaktion einzugehen, wenn der besagte Brei durch nahezu die gesamte Reaktionszone hindurch transportiert wird (62), wodurch eine weitere nahezu einheitliche Lignin-Extraktion eines erheblichen Teils des Breis erhalten wird.

2. Verfahren nach Anspruch 1, welches Verfahren eine chemische Erschließung des Lignin-Zellstoff-Materials durch Kraft-Breierstellung, Kraft-AQ-Breierstellung oder durch eine verlängerte Lignin-Extraktion umfaßt.

3. Verfahren nach Anspruch 1 oder 2, wobei der Sauerstoff-Lignin-Extraktionsschritt die Erstellung eines Breis mit niedrigere bis durchschnittlicher Konsistenz umfaßt; die Behandlung des Breis mit niedrigere bis durchschnittlicher Konsistenz mit wäßriger Lösung eines alkalischen Materials während einer bestimmten Dauer und bei einer bestimmten Temperatur, je nach der Menge des alkalischen Materials, um das alkalische Material gleichmäßig auf den Brei mit niedriger bis durchschnittlicher Konsistenz zu verteilen; die Erhöhung der Konsistenz des Breis auf einen hohen wert von 20% bis 50% und wobei der daraus sich ergebende Brei mit hoher Konsistenz einer Sauerstoff-Lignin-Extraktion für hohe Konsistenz unterzogen wird, um den Übergangsbrei zu realisieren.

4. Verfahren nach Anspruch 1, 2 oder 3, wobei die letztendliche GE-Klarheit des gebleichten Breis wenigstens 50% beträgt und die Viskosität größer als etwa 10 cps ist und wobei die Ligninmenge durch eine K-Nr. des Übergangsbreis von etwa 10 oder weniger gegeben ist und wobei die Viskosität des Übergangsbreis größer als etwa 13 cps ist.

5. Verfahren nach Anspruch 1, 2, 3 oder 4, wobei das Lignin-Zellstoff-Material "softwood" ist und die letztendliche GE-Klarheit des gebleichten Breis wenigstens etwa 50% beträgt und dessen Viskosität größer als etwa 10 cps ist und wobei die Menge Lignin von einer K-Nummer des Übergangsbreis gegeben ist, die zwischen etwa 7 und 10 gelegen ist, und die Viskosität des Übergangsbreis größer als etwa 13 cps ist.

6. Verfahren nach Anspruch 1, 2, 3, 4 oder 5, wobei das Lignin-Zellstoff-Material "Hardwood" ist und die letztendliche GE-Klarheit des gebleichten Breis wenigstens 55% beträgt und dessen Viskosität größer als etwa 10 cps ist und wobei die Ligninmenge mit einer K-Nr. des Übergangsbreis angegeben wird, die zwischen etwa 5 und 8 gelegen ist, und die Viskosität des Übergangsbreis größer als etwa 13 cps ist.

7. Verfahren nach Anspruch 4, 5 oder 6, wobei die Lignin-Menge, die sich im Brei befindet, nach der Lignin- Extraktion durch Ozon, von einer K-Nr. eines gebleichten Breis von etwa 3 bis 4 wiedergegeben wird.

8. Verfahren nach Anspruch 1, weiter das Bleichen des Breis nach der Ozon-Lignin-Extraktion mit einem Klarheitssteigernden Agens umfassend, um die GE-Klarheit des gebleichten Breis zu steigern.

9. Verfahren nach Anspruch 8, weiter die Kombination des gebleichten Breis mit einer wirksamen Menge eines alkalischen Materials in einer alkalischen wäßrigen Lösung bei einer Temperatur umfassend, die mit der Menge des alkalischen Materials im Zusammenhang steht, um einen erheblichen Teil von jeglichem Lignin, das in dem gebleichten Brei zurückgeblieben ist, in Lösung zu bringen, wonach eine Extraktion eines Teils der wäßrigen alkalischen Lösung folgt, um nahezu sämtliches in Lösung gebrachtes Lignin daraus zu entfernen und einen extrahierten Brei zu erstellen, bevor mit dem klarheitssteigernden Agens gebleicht wird.

10. Verfahren nach Anspruch 8, wobei das klarheitssteigernde Agens Chlordioxid oder ein Peroxid ist.

11. Verfahren nach Anspruch 1, wobei das Lignin-Zellstoff- Material chemisch erschlossen wird, um einen Brei mit einer ersten K-Nr. und einem ersten Viskositätswert zu bilden, wonach der Brei einer Lignin-Extraktion mit Sauerstoff unterzogen wird, um einen teilweise von Lignin befreiten Brei mit einer zweiten K-Nr., die unter der bereits genannten ersten K-Nr. liegt, zu bilden, dazu ausreichend, um den teilweise durch Lignin-Extraktion erhaltenen Brei weiter mit Ozon zu extrahieren, unter Beibehaltung der Viskosität auf einem derartigen Niveau, daß die Zellstoff-Komponenten dieses teilweise von Lignin befreiten Breis nicht in erheblichem Umfange von der Sauerstoff-Lignin-Extraktion befallen werden; und der teilweise von Lignin befreite Brei durch das Ozon weiter von Lignin befreit wird, um einen zum Großteil ligninfreien Brei mit einer dritten K-Nummer zu bekommen, die erheblich unter der der zweiten K-Nr. des bereits genannten teilweise ligninbefreiten Breis gesunken ist, und welcher Brei einen GE-Klarheitswert hat, der erheblich über dem des teilweise ligninbefreiten Breis gelegen ist, dies unter Erhalt der Viskosität und ohne einen aggressiven chemischen Angriff auf die Zellstoffkomponenten des Breis, um zum Großteil eine Herabsetzung der Konsistenz des Breis zu vermeiden.

12. Verfahren nach Anspruch 11, in der der teilweise von Lignin befreite Brei eine Menge Lignin enthält, die es ermöglicht, daß nach der Ozon-Lignin-Extraktion der Brei die bestimmte GE-Klarheit bekommt und ebenfalls eine Viskosität hat, die ausreichend hoch ist, um den Viskositätsrückgang bei der Ozon-Lignin-Extraktion auszugleichen, wodurch der nahezu ligninfreie Brei die bestimmte Konsistenz erhalten kann.

13. Verfahren nach Anspruch 11, weiter die Kombination des nahezu ligninfreien Breis und einer effektiven menge alkalischen Materials in einer alkalisch wäßrigen Lösung bei einer bestimmten von der gesamten Menge alkalischen Materials abhängigen Temperatur umfassend, um einen erheblichen Teil des Lignins, das möglicherweise noch in dem nahezu ligninfreien Brei zurückgeblieben ist, in Lösung zu bringen und danach einen Teil der wäßrigen alkalischen Lösung zu extrahieren, um auf diese Weise nahezu sämtliches in Lösung gebrachte Lignin daraus zu entfernen und einen nahezu ligninfreien Brei zu realisieren.

14. Verfahren nach Anspruch 13, weiter das Bleichen des nahezu ligninfreien Breis zu einem Klarheitswert umfassend, der erheblich über dem des nahezu ligninfreien Breis gelegen ist.

15. Verfahren nach Anspruch 11, wobei die Viskosität des genannten nahezu ligninfreien Breis auf einem wert von mehr als etwa 13 cps gehalten wird.

16. Verfahren nach Anspruch 15, wobei der genannte teilweise ligninfreie Brei auf einer Viskositätsabnahme von etwa 30% oder weniger gegenüber dem erstgenannten Wert gehalten wird.

17. Verfahren nach Anspruch 11, wobei das Lignin-Zellstoff-Material ein "Hardwood" ist.

18. Verfahren nach Anspruch 17, wobei die genannte erste K-Nr. zwischen etwa 10 und 14 gelegen ist.

19. Verfahren nach Anspruch 17, wobei der genannte erste Viskositätswert zwischen 21 und 18 cps gelegen ist.

20. Verfahren nach Anspruch 17, wobei die genannte zweite K-Nr. zwischen etwa 5 und 8 gelegen ist.

21. Verfahren nach Anspruch 20, wobei die genannte dritte K-Nr. kleiner als etwa 5 ist.

22. Verfahren nach Anspruch 11, wobei das genannte Lignin- Zellstoff-Material ein "Softwood" ist.

23. Verfahren nach Anspruch 22, worin die erste genannte K-Nr. zwischen 20 und 24 gelegen ist.

24. Verfahren nach Anspruch 22, worin die genannte zweite K-Nr. zwischen etwa 7 und 10 gelegen ist.

25. Verfahren nach Anspruch 11, wobei die Sauerstoff-Lignin-Extraktionsbehandlung auf einen Brei mit durchschnittlicher Konsistenz durchgeführt wird.

26. Verfahren nach Anspruch 11, wobei der teilweise Lignin-Extraktionsschritt weiter umfaßt:
die Behandlung des genannten Breis mit einer Menge alkalischen Materials in einer wäßrigen alkalischen Lösung während einer bestimmten Zeit und bei einer bestimmten Temperatur, abhängig von der Menge alkalischen Materials, um damit eine nahezu einheitliche Verteilung des alkalischen Materials in dem Brei zu erhalten;
die Erhöhung der Konsistenz nach der Vollendung des Behandlungsschritts und
die Anwendung einer Sauerstoff-Lignin-Extraktionsbehandlung für hohe Konsistenz auf den alkalisches Material enthaltenden Brei mit erhöhter Konsistenz, um einen teilweise ligninfreien Brei zu realisieren.

27. Verfahren nach Anspruch 11, wobei die Viskosität des genannten nahezu ligninfreien Breis auf einem wert von mehr als 10 cps gehalten wird.

28. Verfahren nach Anspruch 27, wobei der genannte nahezu lignin-freie Brei auf einer Viskositätsabnahme von etwa 30 % oder weniger gegenüber der Viskosität des genannten nahezu ligninfreien Breis gehalten wird.

29. Verfahren nach Anspruch 11, wobei der weitere Lignin-Extraktionsschritt zusätzlich umfaßt:
die Erhöhung der Konsistenz des genannten teilweise ligninfreien Breis;
die Zerkleinerung des Breis mit erhöhter Konsistenz auf eine vorher festgelegte Teilchengröße; und
das gleichmäßige Berührenlassen des Breis mit zerkleinerten Teilchen mit der genannten effektiven menge Ozon, wenn der Brei im Laufe des Verfahrens fortschreitet.

30. Verfahren nach Anspruch 29, wobei die Teilchengröße des Breis mit erhöhter Konsistenz derart verkleinert wird, daß ein einheitlicher Kontakt mit dem Ozon erleichtert wird, ohne einen erheblichen Rückgang der Zellstoffkomponenten des Breis zu verursachen.

31. Verfahren nach Anspruch 30, wobei der Brei auf etwa 5 mm zerkleinert wird und den Prozeß in der Weise durchläuft, daß eine nicht-gleichmäßige Bearbeitung des Breis durch das Ozon vermieden wird.

32. Verfahren nach Anspruch 31, wobei der zerkleinerte Brei in derselben Richtung wie das Ozon fließt.

33. Verfahren nach Anspruch 31, wobei der zerkleinerte Brei im Gegenstrom zum Ozon fließt.

34. Verfahren nach Anspruch 14, wobei der nahezu ligninfreie Brei mit Chlordioxid gebleicht wird.

35. Verfahren nach Anspruch 14, wobei der nahezu ligninfreie Brei mit einem Peroxid gebleicht wird.

36. Verfahren nach Anspruch 34 oder 35, wobei das Bleichen die GE-Klarheit des genannten nahezu ligninfreien Breis auf wenigstens etwa 70% erhöht.

37. Verfahren nach Anspruch 34 oder 35, wobei die Bleichbearbeitung die GE-Klarheit des nahezu ligninfreien Breis auf wenigstens etwa 80% erhöht.

38. Verfahren nach Anspruch 34 oder 35, wobei die Bleichbearbeitung die GE-Klarheit des nahezu ligninfreien Breis auf wenigstens etwa 90% erhöht.

39. Verfahren nach Anspruch 1, wobei der Brei, der durch Sauerstoff-Lignin-Extraktion erhalten worden ist, eine K- Nr. von etwa 10 oder weniger und eine Viskosität von mehr als etwa 134 cps nach der Sauerstoff-Lignin-Extraktion hat, und der Brei, der durch die Ozon-Lignin-Extraktion erhalten worden ist, eine K-Nr. von ungefähr 5 oder weniger und eine Viskosität von mehr als etwa 10 und eine GE-Klarheit von wenigstens etwa 50% nach der Ozon-Lignin-Extraktion hat.

40. Verfahren nach Anspruch 39, wobei das Lignin-Zellstoff-Material ein "Softwood" ist und einer teilweisen Ligninextraktion unterzogen wird, bis der Brei eine K-Nr. von etwa 7 bis 10 und eine Viskosität von mehr als etwa 13 hat, vor der Ligninextraktion mit Ozon.

41. Verfahren nach Anspruch 40, wobei der "Softwood"_Brei eine K-Nr. von etwa 3 bis 4 hat, und eine Viskosität von mehr als etwa 10 und eine GE-Klarheit von wenigstens etwa 50% nach der weiteren Lignin-Extraktion mit Ozon.

42. Verfahren nach Anspruch 39, wobei das Lignin-Zellstoff-Material ein "Hardwood" ist und teilweise von Lignin zu einem Brei mit einer K-Nr. von etwa 5 bis 8 und einer Viskosität von mehr als etwa 13 befreit ist, vor der weiteren Lignin-Extraktion mit Ozon.

43. Verfahren nach Anspruch 42, wobei der "Hardwood"-Brei eine K-Nr. von etwa 3 bis 4 und eine Viskosität von mehr als 10 und eine GE-Klarheit von wenigstens etwa 55% hat, nach der weiteren Lignin-Extraktion mit Ozon.

44. Verfahren nach Anspruch 39, weiter umfassend: das Zusammenbringen des nahezu ligninfrei gemachten Breis mit einer wirksamen Menge eines alkalischen Materials in einer wäßrigen alkalischen Lösung während einer bestimmten Zeit und bei einer bestimmten Temperatur, je nach der Menge des alkalischen Materials, um einen erheblichen Teil des im Brei zurückgebliebenen Lignins in Lösung zu bringen, und daran anschließendes Extrahieren eines Teils der wäßrigen alkalischen Lösung, um somit nahezu sämtliches gelöste Lignin daraus zu entfernen und einen nahezu ligninfreien Brei zu realisieren.

45. Verfahren nach Anspruch 44, wobei der genannte Extraktionsschritt die Klarheit des Breis mit etwa 2% erhöht.

46. Verfahren nach Anspruch 44, weiter das Bleichen des nahezu lignin-freien Breis mit Chlordioxid oder mit einem Peroxid umfassend, um die GE-Klarheit auf wenigstens 70% zu steigern.

47. Verfahren nach Anspruch 46, wobei die GE-Klarheit auf wenigstens etwa 80% erhöht wird.

48. Verfahren nach Anspruch 46, wobei die GE-Klarheit auf wenigstens etwa 90% erhöht wird.

49. Verfahren nach Anspruch 44, wobei das Lignin-Zellstoff-Material teilweise durch eine Sauerstoff-Lignin-Extraktionsbehandlung von Lignin befreit wird.

50. Verfahren nach Anspruch 49, wobei die Sauerstoff-Lignin-Extraktionsbehandlung auf einen Brei mit durchschnittlicher Konsistenz durchgeführt wird.

51. Verfahren nach Anspruch 44, wobei das Lignin-Zellstoff-Material teilweise von Lignin befreit wird durch: die Bildung eines Breis mit relativer geringer Konsistenz von weniger als 10 Gew.%;
die Behandlung des Breis mit geringer Konsistenz mit einer Menge alkalischen Materials in einer wäßrigen alkalischen Lösung während einer bestimmten Zeit und bei einer bestimmten Temperatur, je nach der Menge des alkalischen Materials, bis eine nahezu vollständige und zum Großteil gleichmäßige Verteilung des alkalischen Materials im Brei erhalten wird;
die Erhöhung der Konsistenz des Breis auf wenigstens etwa 20 Gew.% nach der Fertigstellung des Behandlungsschritts; und die Anwendung einer Sauerstoff-Lignin-Extraktion für hohe Konsistenz auf den alkalisches Material enthaltenden Brei mit erhöhter Konsistenz, um einen teilweise von Lignin befreiten Brei mit einer K-Nr. von etwa 9 oder weniger und einer Viskosität von etwa 13 oder mehr zu erhalten.

52. Verfahren nach Anspruch 1, wobei der Sauerstoff-Lignin-Extraktionsschritt umfaßt:
die Herabsetzung der Konsistenz des Breis auf eine Konsistenz von weniger als 10 Gew.%;
die Behandlung des Breis mit reduzierter Konsistenz mit einer Menge alkalischen Materials in einer alkalischen wäßrigen Lösung während einer bestimmten Dauer und bei einer bestimmten Temperatur, je nach der Menge des alkalischen Materials, um auf diese Weise praktisch eine nahezu einheitliche Verteilung des alkalischen Materials in dem Brei zu realisieren;
die Erhöhung der Konsistenz des Breis auf wenigstens etwa 20 Gew.% nach der Vervollständigung des Behandlungsschritts; und die Anwendung eines Sauerstoff-Lignin-Extraktionsschritts für höhere Konsistenz auf den alkalisches Material enthaltenden Brei mit erhöhter Konsistenz, um einen teilweise von Lignin befreiten Brei mit einer K-Nr. von etwa 9 oder weniger und einer Viskosität von etwa 13 cps zu erhalten;
die Erstellung durch den Sauerstoff-Lignin- Extraktionsschritt eines erheblichen lignin-freien Breis mit einer K-Nr. von etwa 5 oder weniger, mit einer Viskosität von mehr als etwa 10 und einer GE-Klarheit von wenigstens etwa 50%;
wobei das Verfahren weiter umfaßt:
die Kombination des mit Ozon von Lignin befreiten Breis, mit einer effektiven Menge alkalischen Materials in einer wäßrigen alkalischen Lösung während einer bestimmten Dauer und bei einer bestimmten Temperatur, abhängig von der Menge alkalischen Materials, um einen erheblichen Teil des gegebenenfalls in dem Brei zurückgebliebenen Lignins in Lösung zu bringen;
die Extraktion eines Teils der wäßrigen Lösung, um somit nahezu sämtliches in Lösung gebrachtes Lignin daraus zu entfernen und nahezu ligninfreien Brei zu realisieren; und
das Bleichen des nahezu ligninfreien Breis, um die GE- Klarheit auf wenigstens etwa 70% zu erhöhen.

53. Verfahren nach Anspruch 52, wobei die GE-Klarheit auf wenigstens 80% erhöht wird.

54. Verfahren nach Anspruch 52, wobei die GE-Klarheit auf wenigstens 90% erhöht wird.

55. Verfahren nach Anspruch 52, wobei das Lignin-Zellstoff-Material ein "Softwood" ist und teilweise von Lignin auf eine K-Nr. von etwa 8 bis 9 und eine Viskosität von mehr als etwa 14 vor der weiteren Lignin-Extraktion mit Ozon befreit wird.

56. Verfahren nach Anspruch 55, wobei das "Softwood" eine K-Nr. zwischen etwa 3 und 4, eine Viskosität von etwa 10 und eine GE-Klarheit von wenigstens etwa 54 %nach der weiteren Lignin-Extraktion mit Ozon hat.

57. Verfahren nach Anspruch 52, wobei das Lignin-Zellstoff-Material ein "Hardwood" ist und teilweise von Lignin zu einem Brei mit einer K-Nr. von etwa 6 bis 7 und einer Viskosität von mehr als etwa 15 befreit ist, bevor die weiteren Lignin-Extraktion mit Ozon stattfindet.

58. Verfahren nach Anspruch 57 wobei der "Hardwood"-Brei eine K-Nr. von etwa 3 bis 4 und eine Viskosität von mehr als 10 und eine GE-Klarheit von wenigstens etwa 63% hat, nach dem genannten Lignin-Extraktionsschritt mit Ozon.

59. Verfahren nach Anspruch 52, wobei das teilweise von Lignin befreite Lignin-Zellstoff-Material durch Kraft-Breierstellung, Kraft-AQ-Breierstellung oder durch einen verlängerten Lignin-Extraktionsschritt eines Lignin-Zellstoffmaterials erhalten worden ist.

60. Verfahren nach Anspruch 52, welches Verfahren die Herabsetzung der K-Nr. des Breis mit erhöhter Konsistenz um wenigstens etwa 60% während des Sauerstoff-Lignin Extraktionsschritts umfaßt, ohne dabei die Zellstoffkomponenten des Breis erheblich zu beschädigen.

61. Verfahren nach Anspruch 52, wobei der Brei einem Sauerstoff-Lignin-Extraktionsschritt bei hoher Konsistenz unterzogen wird, ohne in erheblichem Umfange die Viskosität des Breis zu verändern.

62. Verfahren nach Anspruch 52, welches Verfahren die Herabsetzung des Verhältnisses der K-Nr. gegenüber der Viskosität des Breis während des Sauerstoff-Lignin- Extraktionsschritts um wenigstens 25% umfaßt.

63. Verfahren nach Anspruch 52, wobei die Konsistenz des Breis, der mit der wäßrigen alkalischen Lösung behandelt ist, vor dem Sauerstoff-Lignin-Extraktionsschritt zwischen etwa 1 und 4,5 Gew.% gelegen ist.

64. Verfahren nach Anspruch 52, wobei die Konsistenz des Breis auf etwa 25 bis 35 Gew-% erhöht worden ist, vor Ausführung des Sauerstoff-Lignin-Extraktionsschritts.

65. erfahren nach Anspruch 52, wobei die Menge alkalischen Materials, verteilt auf den Brei mit geringer Konsistenz vor der Sauerstoff-Lignin-Extraktion zwischen etwa 15 und 30 Gew.% gegenüber dem Trockengewicht des Breis liegt.

66. Verfahren nach Anspruch 65, wobei die wäßrige alkalische Lösung eine Konzentration an alkalischem Material hat, gelegen zwischen etwa 20 und 120 g/l, so daß die Konzentration des alkalischen Materials im Brei mit niedriger Konzentration zwischen 6,5 und 13 g/l liegt.

67. Verfahren nach Anspruch 52, wobei der alkalische Behandlungsschritt während einer Zeit durchgeführt wir,d die zwischen etwa 1 und 5 Minuten gelegen ist, bei einer Temperatur, die zwischen etwa 90 und 150°F liegt.

68. Verfahren nach Anspruch 52, wobei der ursprünglich gebildete Brei ein "Brownstock"_Brei ist und wobei weiter wenigstens ein Teil der Flüssigkeit, erhalten aus der alkalischen Lösung in dem Schritt vor der Erhöhung der Konsistenz des Breis in den alkalischen Behandlungsschritt zurückgeführt wird.

69. Verfahren nach Anspruch 1, wobei:
der Brei ursprünglich als ein "Brownstock"-Brei mit einer K-Nr. zwischen etwa 10 und 24 durch Kraft-Breierstellung, Kraft-AQ-Breierstellung oder durch eine verlängerte Lignin-Extraktion des Lignin-Zellstoff-Materials gebildet wird;
die Sauerstoff-Lignin-Extraktionsschritt umfaßt;
die Herabsetzung der Konsistenz des genannten Breis auf etwa 1 bis 4,5 Gew.%;
Behandlung des Breis mit verringerter Konsistenz mit einer Menge alkalischen Materials in einer wäßrigen alkalischen Lösung mit einer Konzentration des alkalischen Materials zwischen etwa 20 und 120 g/l während einer Zeit, die zwischen etwa 1 und 15 Minuten liegt, und bei einer Temperatur, gelegen zwischen 90° und 150°F, dies in der Weise, daß die Konzentration des alkalischen Materials im Brei mit verringerter Konsistenz während dieses Behandlungsschritts zwischen 6,5 und 13 g/l liegt, um auf diese Weise eine nahezu einheitliche Verteilung des alkalischen Materials in dem Brei zu vervollständigen;
die Erhöhung der Konsistenz des alkalisch behandelten Breis auf etwa 25 bis 35 Gew.%;
die Anwendung einer Sauerstoff-Lignin-Extraktion für hohe Konzentration auf den Brei mit erhöhter Konsistenz, ohne die Viskosität des Breis in erheblichem Umfange zu ändern und somit einen teilweise lignin-freien Brei zu realisieren mit einer K-Nr. von etwa 10 oder weniger und einer Viskosität von mehr als etwa 13, wobei das Verhältnis der K-Nr. zu der Viskosität des genannten Breis während der Sauerstoff-Lignin-Extraktion um wenigstens 25% herabgesetzt wird;
wobei der Ozon-Lignin-Extraktionsschritt einen zum Großteil ligninfreien Brei ergibt mit einer K-Nr. von etwa 5 oder weniger, mit einer Viskosität von mehr als etwa 10 und mit einer GE-Klarheit von wenigstens etwa 50%;
wobei der Prozeß weiter umfaßt:
die Kombination des zum Großteil ligninfreien Breis mit einer wirksamen Menge alkalischen Materials in einer wäßrigen alkalischen Lösung während einer bestimmten Zeit und bei einer bestimmten Temperatur, abhängig von der Menge alkalischen Materials, um einen erheblichen Teil des Lignins, das in dem Brei zurückgeblieben ist, in Lösung zu bringen;
die Extraktion eines Teils der wäßrigen alkalischen Lösung, um somit nahezu sämtliches in Lösung gebrachtes Lignin daraus zu entfernen und einen nahezu ligninfreien Brei zu realisieren; und das Bleichen des nahezu ligninfreien Breis, um die GE- Klarheit auf wenigstens etwa 70% zu erhöhen.

70. Verfahren nach Anspruch 69, wobei die GE-Klarheit auf wenigstens etwa 80% erhöht wird.

71. Verfahren nach Anspruch 69, wobei die GE-Klarheit auf wenigstens etwa 90% erhöht wird.

72. Verfahren nach Anspruch 69, welches die Herabsetzung der K-Nr. des Breis mit erhöhter Konsistenz um wenigstens etwa 60% während des Sauerstoff-Lignin- Extraktionsschritts umfasst, ohne dabei die Zellstoffkomponenten des Breis in erheblichem Umfange zu beschädigen.

73. Verfahren nach Anspruch 69, wobei der nahezu ligninfreie Brei mit Chlordioxid oder mit einem Peroxid gebleicht wird.

74. Verfahren nach Anspruch 73, wobei das Peroxid Wasserstoffperoxid ist.

75. Verfahren nach Anspruch 69, weiter umfassend die Hinzufügung eines chelatbildenden Stoffs zum Brei vor dem Ozon-Lignin- Extraktionsschritt, um Metallionen nahezu nicht-reaktiv gegenüber Ozon zu machen.

76. erfahren nach Anspruch 75, wobei der chelatbildende Stoff DTPA, EDTA oder Oxalsäure ist.

77. Verfahren nach Anspruch 69, weiter umfassend die Einstellung vor dem Ozon-Lignin-Extraktionsschritt des pH-Werts des Breis bis in einen Bereich von 1 bis 4, durch Hinzufügen einer ausreichenden Menge Säurematerials zum Brei.

78. Verfahren nach Anspruch 69, weiter umfassend die Erhöhung Lignin-Extraktionsschritt der Konsistenz des Breis auf einen Wert, der zwischen etwa 25 und 50 Gew.% liegt vor dem Ozon.

79. Verfahren nach Anspruch 78, wobei vor dem Ozon-Lignin-Extraktionsschritt die Konsistenz des Breis auf einen Wert erhöht wird, der zwischen etwa 35 und 45 Gew.% liegt.

80. Verfahren nach Anspruch 69, welches Verfahren die Zerkleinerung des Breis zu einem Durchmesser von weniger als etwa 5 mm nach dem Sauerstoff-Lignin Extraktionsschritt und vor dem Ozon-Lignin- Extraktionsschritt umfaßt.

81. Verfahren nach Anspruch 69, welches Verfahren weiter umfaßt, daß der Brei auf einer Temperatur von weniger als etwa 120°F während des Ozon-Lignin-Extraktionsschritts gehalten wird.

82. Verfahren nach Anspruch 69, wobei das Ozon durch eine Gemisch geliefert wird, das Ozon und Sauerstoff enthält.

83. Verfahren nach Anspruch 82, wobei die Ozonkonzentration in dem Gemisch zwischen etwa 1 und 8 Volumen% gelegen ist.

84. Verfahren nach Anspruch 69, wobei das Ozon von einem Gemisch aus Ozon und Luft geliefert wird.

85. Verfahren nach Anspruch 84, wobei die Ozonkonzentration zwischen etwa 1 und 4 Volumen% liegt.

86. Verfahren nach Anspruch 69, welches Verfahren die Beförderung des teilweise ligninfreien Breis während des Ozon-Lignin-Extraktionsschritts umfaßt, dies in der Weise, daß nahezu sämtlicher Brei dem Ozon ausgesetzt wird.

87. Verfahren nach Anspruch 86, wobei das Ozon im Gegenstrom dem fortschreitenden Brei zugeführt wird.

88. Verfahren nach Anspruch 86 wobei das Ozon in derselben Richtung als der fortschreitende Brei fliesst.

89. Verfahren nach Anspruch 1, wobei:
der durch Ozon von Lignin befreite Brei eine K-Nr. von etwa 10 oder weniger und eine Viskosität von mehr als etwa 13 cps hat;
der Ozon-Lignin-Extraktionsschritt umfaßt:
die Hinzufügung eines chelatbildenden Agens zum Brei, um Metallionen davon nahezu nicht-reaktiv gegenüber Ozon zu machen;
die Einstellung des pH-Werts des besagten Breis bis in einen Bereich von etwa 1 bis 4, durch Hinzufügen einer ausreichenden Menge Säurematerials;
die Erhöhung der Konsistenz des genannten Breis auf einen Wert, der zwischen etwa 25 und 50% gelegen ist;
die Zerkleinerung des Breis mit erhöhter Konsistenz bis zu einem Durchmesser von weniger als etwa 5 mm; und
die Extraktion des Lignins aus dem genannten Brei mit erhöhter Konsistenz mit einer effektiven Menge Ozon während einer ausreichenden Dauer, indem der zerkleinerte Brei in der Weise befördert wird, daß nahezu sämtlicher Brei dem Ozon ausgesetzt wird, um einen Brei zu bekommen, der erheblich weniger Lignin enthält und der eine K-Nr. von ungefähr 5 oder weniger und eine Viskosität von mehr als etwa 10 sowie eine GE-Klarheit von wenigstens etwa 50% hat;
welches Verfahren weiter umfaßt:
das Zusammenbringen des zum Großteil ligninfreien Breis mit einer effektiven Menge alkalischen Materials in einer wäßrig alkalischen Lösung während einer bestimmten Zeit und bei einer bestimmten Temperatur, abhängig von der Menge alkalischen Materials, um einen erheblichen Teil des Lignins, das gegebenenfalls in dem Brei zurückgeblieben ist, in Lösung zu bringen;
die Extraktion eines Teils der wäßrigen alkalischen Lösung, um auf diese Weise nahezu alles in Lösung gegangene Lignin daraus zu entfernen und einen nahezu ligninfreien Brei zu realisieren; und
das Bleichen des nahezu ligninfreien Breis mit Chlordioxid, um dessen GE-Klarheit auf wenigstens etwa 70% zu erhöhen.

90. Verfahren nach Anspruch 89, wobei die GE-Klarheit auf wenigstens etwa 80% erhöht wird.

91. Verfahren nach Anspruch 89, wobei die GE-Klarheit auf wenigstens etwa 90% erhöht wird.

92. Verfahren nach Anspruch 89, wobei der Breierstellungsschritt eine Kraft-Breierstellung umfaßt und der sauerstoff-Lignin-Extraktionsschritt die K-Nr. des Breis um wenigstens etwa 60% herabsetzt, ohne die Zellstoffkomponenten des Breis erheblich zu beschädigen oder ohne die Viskosität des Breis erheblich zu ändern.

93. Verfahren nach Anspruch 92, wobei der Breierstellungsschritt eine Kraft-AQ-Breierstellung umfaßt.

94. Verfahren nach Anspruch 93, wobei der Breierstellungsschritt die K-Nr. des Breis um wenigstens etwa 60% herabsetzt, ohne dabei die Zellstoffkomponenten des Breis in erheblichem Umfange zu beschädigen oder die Viskosität in erheblichem Umfange zu ändern.

95. Verfahren nach Anspruch 89, wobei der Breierstellungsschritt die Kombination der Kraft-AQ-Breierstellung und der verlängerten Lignin-Extraktion umfaßt und der sauerstoff-Lignin-Extraktionsschritt die K- N r. des Breis um wenigstens in etwa 60% herabsetzt, ohne die Zellstoffkomponenten des Breis in erheblichem Umfange zu beschädigen oder ohne die Viskosität des Breis in erheblichem Umfange zu ändern.

96. Verfahren nach Anspruch 89, wobei während der Ozon-Lignin-Extraktion der Brei in der Weise befördert wird, daß der Brei auf einer Temperatur von weniger als etwa 120°F gehalten wird.

97. Verfahren nach Anspruch 89, wobei das chelatbildende Agens und die Säure dem Brei in einer Mischkammer beigefügt werden.

98. Verfahren nach Anspruch 97, wobei wenigsten ein Teil der Flüssigkeit, der bei dem Schritt zur Erhöhung der Konzentration von dem Brei abgetrennt ist, der Mischkammer zugeführt wird.

99. Verfahren nach Anspruch 97, wobei der Brei in derselben Richtung wie das Ozon befördert wird.

100. Verfahren nach Anspruch 97, wobei der Brei im Gegenstrom zum Ozon befördert wird.

101. Verfahren nach Anspruch 1, wobei:
der durch Sauerstoff von Lignin befreite Brei eine K-Nr. von ungefähr 10 oder weniger und eine Viskosität von mehr als etwa 13 cps hat;
der Ozon-Lignin-Extraktionsschritt umfaßt:
die Hinzufügung eines chelatbildenden Agens zu dem Brei, um darin Metallionen praktisch nicht -reaktiv gegenüber Ozon zu machen;
die Einstellung des pH-Wertes des Breis auf einen Wert von etwa 1 bis 4, durch Hinzufügen einer ausreichenden menge Säurematerials;
die Erhöhung der Konsistenz des Breis auf einen Wert, der zwischen etwa 25 und 50% gelegen ist;
die Zerkleinerung des Breis mit erhöhter Konsistenz auf einen Durchmesser von weniger als etwa 5 mm;
die Extraktion des Lignins aus dem Brei mit erhöhter Konsistenz mittels einer effektiven Menge Ozons während einer ausreichenden Dauer, um einen zum Großteil von Lignin befreiten Brei mit einer K-Nr. von etwa 5 oder weniger, einer Viskosität von mehr als etwa 10 und einer GE-KLarheit von wenigstens etwa 50% zu realisieren;
welches Verfahren weiter umfaßt:
die Kombination des in erheblichem Umfange von Lignin befreiten Breis mit einer wirksamen Menge alkalischen Materials in einer wäßrigen alkalischen Lösung während einer bestimmten Zeit und bei einer bestimmten Temperatur, abhängig von der Menge alkalischen Materials, um einen erheblichen Teil des Lignins, das in dem Brei zurückgeblieben ist, in Lösung zu bringen;
die Extraktion eines Teils der wäßrigen alkalischen Lösung, um somit nahezu sämtliches in Lösung gebrachtes Lignin daraus zu entfernen und einen nahezu ligninfreien Brei zu realisieren; und
das Bleichen des nahezu ligninfreien Breis, um die GE- Klarheit auf wenigstens etwa 70% zu erhöhen.

102. Verfahren nach Anspruch 101, wobei die GE-Klarheit auf wenigstens etwa 80% erhöht wird.

103. Verfahren nach Anspruch 101, wobei die GE-Klarheit auf wenigstens etwa 90% erhöht wird.

104. Verfahren nach Anspruch 101, wobei der Breierstellungsschritt eine Kraft-Breierstellung umfaßt und der Sauerstoff-Lignin-Extraktionsschritt die K-Nr. des Breis um wenigstens etwa 60% herabsetzt, ohne die Zellstoffkomponenten des Breis erheblich zu beschädigen oder ohne die Viskosität des Breis erheblich zu ändern.

105. Verfahren nach Anspruch 101, wobei der Breierstellungsschritt eine Kraft-AQ-Breierstellung umfaßt.

106. Verfahren nach Anspruch 105, wobei der Breierstellungsschritt die K-Nr. des Breis um wenigstens etwa 60% herabsetzt, ohne dabei die Zellstoffkomponenten des Breis in erheblichem Umfange zu beschädigen oder die Viskosität des Breis in erheblichem Umfange zu ändern.

107. Verfahren nach Anspruch 101, wobei der Breierstellungsschritt die Kombination der Kraft-AQ-Breierstellung und der verlängerten Lignin-Extraktion umfaßt und der Sauerstoff-Lignin-Extraktionsschritt die K- Nr. des Breis um wenigstens etwa 60% herabsetzt, ohne die Zellstoffkomponenten des Breis in erheblichem Umfange zu beschädigen oder ohne die Viskosität des Breis in erheblichem Umfange zu ändern.

108. Verfahren nach Anspruch 89 oder Anspruch 101, wobei die Ozon-Lignin-Extraktion die K-Nr. des Breis um wenigstens 50% herabsetzt.

109. Verfahren nach Anspruch 89 der 101 wobei die GE-Klarheit des Breis um wenigstens 50% erhöht wird.

110. Verfahren nach Anspruch 109, wobei die GE-Klarheit des Breis auf wenigstens 83% erhöht wird.

111. Verfahren nach Anspruch 1, wobei:
der Brei zwischen dem chemischen Erschließungsschritt und dem Sauerstoff-Lignin-Extraktionsschritt gewaschen wird, wobei der Brei nach dem Sauerstoff-Lignin Extraktionsschritt eine K-Nr. von ungefähr 10 oder weniger und eine Viskosität von mehr als etwa 13 cps hat;
und das Verfahren weiter umfaßt:
das Waschen des mit Sauerstoff von Lignin befreiten Breis; die Fortsetzung des Ozon-Lignin-Extraktionsschritts zum Erhalt eines in erheblichem Umfange von Lignin befreiten Breis mit einer K-Nummer von etwa 5 oder weniger, mit einer Viskosität von mehr als ungefähr 10 und einer GE-Klarheit von wenigstens etwa 50%;
das Waschen des in hohem Maße von Lignin befreiten Breis;
die Kombination des in hohem Maße von Lignin befreiten Breis und einer effektiven Menge alkalischen Materials in einer wäßrigen alkalischen Lösung während einer bestimmten Zeit und bei einer bestimmten Temperatur, abhängig von der gesamten Menge alkalischen Materials, um einen erheblichen Teil des Lignins, das möglicherweise noch in dem nahezu ligninfreien Brei zurückgeblieben ist, in Lösung zu bringen;
die Extraktion eines Teils der wäßrigen alkalischen Lösung, um auf diese Weise nahezu sämtliches in Lösung gebrachtes Lignin daraus zu entfernen und einen im wesentlichen ligninfreien Brei zu realisieren;
das Waschen des im wesentlichen ligninfreien Breis;
das Bleichen des im wesentlichen ligninfreien Breis mit Chlordioxid oder einem Peroxid, um die GE-Klarheit zu erhöhen auf wenigstens etwa 70%; und
das Waschen des gebleichten Breis.

112. Verfahren nach Anspruch 111, wobei die GE-Klarheit auf wenigstens etwa 80% erhöht wird.

113. Verfahren nach Anspruch 111, wobei die GE-Klarheit auf wenigstens etwa 90% erhöht wird.

114. Verfahren nach Anspruch 111, wobei die Waschbearbeitung vor dem Bleichen des Breis umfaßt: das Waschen des Breis mit Frischwasser und die Abtrennung des Breis aus dem ausfließenden Waschwasser.

115. Verfahren nach Anspruch 111, worin beim Bleichschritt Chlordioxid verwendet wird und das ausfließende vom Brei stammende Waschwasser abgeführt wird.

116. Verfahren nach Anspruch 111, worin bei der Bleichbearbeitung Chlordioxid verwendet wird und das ausfließende Waschwasser des gebleichten Breis durch umgekehrte Osmose behandelt wird, um ein behandeltes Filtrat zu bilden, wobei wenigstens ein Teil des gebildeten Filtrats zur Waschbearbeitung des nahezu ligninfreien Breis geführt wird.

117. Verfahren nach Anspruch 111, wobei in der Bleichbearbeitung ein Peroxid verwendet wird und wenigstens ein Teil des gebleichten Breis zu dem Schritt zurückgeführt wird, bei dem der nahezu ligninfreie Brei gewaschen wird.

118. Verfahren nach Anspruch 116 oder 117, wobei die Waschbearbeitung für den nahezu ligninfreien Brei umfaßt: das Waschen des Breis mit Waschwasser, das von dem gebleichten Brei stammt, und die Absonderung des Breis aus dem daraus sich ergebenden Waschwasser und die Rückführung von wenigstens einem Teil des besagten Waschwassers zu der Waschbearbeitung des nahezu ligninfreien Breis.

119. Verfahren nach Anspruch 118, wobei die Waschbearbeitung des nahezu ligninfreien Breis umfaßt: das Waschen des besagten Breis mit dem Waschwasser des nahezu ligninfreien Breis, die Absonderung des Breis aus dem daraus sich ergebenden Waschwasser und die Zuführung von wenigstens einem Teil dieses Waschwassers zu der Waschbearbeitung für den teilweise von Lignin befreiten Brei.

120. Verfahren nach Anspruch 119, wobei die Waschbearbeitung für den teilweise von Lignin befreiten Brei umfaßt: das Waschen des besagten Breis mit Waschwasser des zum Großteil von Lignin befreiten Breis, die Absonderung des Breis aus dem sich daraus ergebenden Waschwasser und die Zuführung von wenigstens einem Teil des besagten Waschwassers zur Waschbearbeitung des Breis.

121. Verfahren nach Anspruch 120, wobei die Waschen des bearbeitung des Breis umfaßt: das Waschend es besagten Breis mit Waschwasser des teilweise von Lignin befreiten Breis, das Absondern des Breis aus dem sich daraus ergebenden Waschwasser, das Sammeln und Konzentrieren des besagten Waschwasser zur Verbrennung in einem Rückgewinnungsboiler.

122. Verfahren nach Anspruch 111 oder 121, wobei in der Bleichbearbeitung Chlordioxid mit einem minimalen Chlorgehalt verwendet wird.

123. Verfahren nach Anspruch 111 oder 121, wobei die erforderliche Menge Wasser für die Waschbearbeitung im Vergleich zu den bekannten CEDED oder IC/DED-Prozessen erheblich verringert wird.

124. Verfahren nach Anspruch 115, wobei die ausfließende Flüssigkeit eine Farbe hat, die nicht stärker als ungefähr 2 Pfund pro Tonne ist, ein BOD5 nicht größer als ungefähr 2 Pfund pro Tonne und eine gesamte Menge organischer Chloride, nicht größer als ungefähr 2.

125. Verfahren nach Anspruch 75, wobei das chelatbildende Agens ein Polykarboxilat oder ein Polykarboxilatderivat ist.

126. Verfahren nach Anspruch 75, wobei das chelatbildende Agens in einer Menge von 0,1 bis 0,2 Gew.% im Vergleich zu ofentrocknem Brei verwendet wird.

127. Verfahren nach Anspruch 75, wobei der Brei auf einen pH-Wert angesäuert wird, der zwischen etwa 1 und etwa 4 vor der Behandlung mit dem chelatbildenden Agens gelegen ist.

128. Verfahren nach Anspruch 75, wobei der Brei nach der Bleichbearbeitung mit Ozon hinsichtlich der Klarheit mit einem Peroxid erhöht wird.

## Revendications

1. Procédé pour la préparation d'une pâte pratiquement uniformément blanchie et formée d'une matière de lignine-cellulose, comprenant la préparation d'une pâte de transition avec une teneur réduite en lignine par la décomposition chimique (4) de la matière de lignine-cellulose suivie d'une décomposition par de l'oxygène (26) de la pâte alors obtenue, lequel procédé se caractérise par les étapes suivantes:
a) le pH de la pâte de transition est réglé (42) dans la plage d'environ 1 à 4.
b) la consistance de la pâte de transition est réglée (48) à une grande valeur d'environ 20 à 50 p.c.
c) la pâte de transition est broyée (56) en des particules discrètes dont la majorité a des dimensions de moins de 5 mm environ.
d) la pâte de transition obtenue après les étapes a), b), c) est soumise à une extraction de lignine en mélangeant la pâte dans un mouvement tourbillonnaire avec une atmosphère de gaz comprenant de l'ozone dans une zone de réaction dynamique (58), et ce pendant un temps et une température suffisants pour la pénétration de l'ozone dans pratiquement toute la pâte de transition afin d'entrer en réaction avec celle-ci, lorsque ladite pâte est transportée (62) à travers presque toute la zone de réaction, ce qui permet d'obtenir une extraction continuée et pratiquement uniforme de la lignine d'une partie considérable de la pâte.

2. Procédé selon la revendication 1 comprenant une décomposition chimique de la matière de lignine-cellulose par la trituration Kraft, la trituration Kraft AQ, ou une extraction de lignine prolongée.

3. Procédé selon la revendication 1 ou 2, l'étape d'extraction oxygène-lignine comprenant la formation d'une pâte de petite à moyenne consistance; le traitement de la pâte ayant une petite à moyenne consistance avec une solution aqueuse d'une matière alcaline pendant un certain temps et à une certaine température dépendant de la quantité de matière alcaline afin de répartir également la matière alcaline dans la pâte de petite à moyenne consistance; l'augmentation de la consistance de la pâte jusqu'à une valeur de 20 p.c. à 50 p.c. et la soumission de la pâte de grande consistance qui en résulte à une extraction oxygène-lignine pour une grande consistance afin de réaliser la pâte de transition.

4. Procédé selon la revendication 1, 2 ou 3, le degré de blancheur GE final de la pâte blanchie étant au moins 50 p.c., sa viscosité étant plus grande que 10 cps environ, la quantité de lignine étant indiquée par un n° K de la pâte de transition d'environ 10 ou moins, et la viscosité de la pâte de transition étant plus grande que 13 cps environ.

5. Procédé selon la revendication 1, 2, 3 ou 4, la matière de ligno-cellulose étant du "softwood" et le degré de blancheur GE final de la pâte blanchie étant au moins 50 p.c., sa viscosité étant plus grande que 10 cps environ, la quantité de lignine étant indiquée par un n° K de la pâte de transition et comprise entre environ 7 et 10, et la viscosité de la pâte de transition étant plus grande que 13 cps environ.

6. Procédé selon la revendication 1, 2, 3, 4 ou 5, la matière de lignine-cellulose étant du "hardwood" et le degré de blancheur GE final de la pâte blanchie étant au moins 55 p.c., sa viscosité étant plus grande que 10 cps environ, la quantité de lignine étant indiquée par un n° K de la pâte de transition et comprise entre environ 5 et 8, et la viscosité de la pâte de transition étant plus grande que 13 cps environ.

7. Procédé selon la revendication 4, 5 ou 6, la quantité de lignine se trouvant dans la pâte après l'extraction de lignine par de l'ozone étant indiquée par un n° K d'une pâte blanchie d'environ 3 à 4.

8. Procédé selon la revendication 1, comprenant ensuite le blanchiment de la pâte après l'extraction ozone-lignine avec un agent augmentant le degré de blancheur afin d'augmenter le degré de blancheur GE de la pâte blanchie.

9. Procédé selon la revendication 8, comprenant ensuite la combinaison de la pâte blanchie avec une quantité effective d'une matière alcaline dans une solution alcaline aqueuse à une certaine température, laquelle est liée à la quantité de matière alcaline, pour dissoudre une partie considérable de toute lignine restée dans la pâte blanchie, après quoi on fait une extraction d'une partie de la solution alcaline aqueuse pour éliminer de la pâte pratiquement toute la lignine déjà dissoute et pour former une pâte extraite avant de blanchir celle-ci avec un agent augmentant le degré de blancheur.

10. Procédé selon la revendication 8, l'agent augmentant le degré de blancheur étant du dioxyde de chlore ou un peroxyde.

11. Procédé selon la revendication 1, la matière de lignine-cellulose étant décomposée chimiquement pour la formation d'une pâte avec un premier n° K et une première valeur de viscosité, après quoi la pâte est soumise à une extraction de lignine avec de l'oxygène pour former une pâte partiellement libérée de lignine avec un deuxième n° K, plus petit que ledit premier n° K et suffisant pour continuer à extraire avec de l'ozone la pâte obtenue partiellement par l'extraction de lignine, avec maintien de la viscosité à un tel niveau que les composants de cellulose de cette pâte partiellement libérée de lignine ne sont pas corrodés chimiquement d'une manière significative par l'extraction oxygène-lignine; et
la pâte partiellement libérée de lignine étant encore libérée de lignine par l'ozone pour obtenir une pâte en grande partie libre de lignine et avec un troisième n° K considérablement réduit en dessous du deuxième n° K de ladite pâte partiellement libérée de lignine et un degré de blancheur GE considérablement plus élevé que celui de la pâte partiellement libérée de lignine avec maintien de la viscosité et sans corrosion chimique agressive des composants de cellulose de la pâte pour éviter en grande partie une réduction de la consistance de la pâte.

12. Procédé selon la revendication 11, la pâte partiellement libérée de lignine comprenant une quantité de lignine qui permet que la pâte après l'extraction de lignine avec de l'ozone obtienne un certain degré de blancheur GE et qu'elle ait également une viscosité qui soit suffisamment grande pour compenser la chute de viscosité lors de l'extraction ozone-lignine, par quoi la pâte pratiquement libre de lignine peut obtenir la consistance désirée.

13. Procédé selon la revendication 11, comprenant ensuite la combinaison d'une pâte pratiquement libre de lignine et une quantité effective d'une matière alcaline dans une solution alcaline aqueuse à une certaine température dépendant de la quantité totale de matière alcaline, pour dissoudre une partie considérable de la lignine possiblement restée dans la pâte pratiquement libre de lignine, et d'extraire ensuite une partie de la solution alcaline aqueuse pour éliminer de la pâte pratiquement toute la lignine déjà dissoute et pour réaliser une pâte pratiquement libre de lignine.

14. Procédé selon la revendication 13, comprenant ensuite le blanchiment de la pâte pratiquement libre de lignine jusqu'à un degré de blancheur qui est considérablement plus grand que celui de la pâte pratiquement libre de lignine.

15. Procédé selon la revendication 11, la viscosité de ladite pâte pratiquement libre de lignine étant maintenue à une valeur plus élevée que 13 cps environ.

16. Procédé selon la revendication 15, ladite pâte pratiquement libre de lignine étant maintenue à une diminution de viscosité d'environ 30 p.c. ou moins de la première valeur mentionnée.

17. Procédé selon la revendication 11, la matière de lignine-cellulose étant un "hardwood".

18. Procédé selon la revendication 17, ledit premier n° K étant compris entre environ 10 et 14.

19. Procédé selon la revendication 17, ladite première valeur de viscosité étant comprise entre 21 et 28 cps.

20. Procédé selon la revendication 17, ledit deuxième n° K étant compris entre environ 5 et 8.

21. Procédé selon la revendication 20, ledit troisième n° K étant plus petit que 5 environ.

22. Procédé selon la revendication 11, ladite matière de lignine-cellulose étant un "softwood".

23. Procédé selon la revendication 22, ledit premier n° K étant compris entre 20 et 24.

24. Procédé selon la revendication 22, ledit deuxième n° K étant compris entre environ 7 et 10.

25. Procédé selon la revendication 11, le traitement d'extraction oxygène-lignine étant appliqué à une pâte ayant une consistance moyenne.

26. Procédé selon la revendication 11,-l'étape d'extraction partielle de lignine comprenant ensuite:
le traitement de ladite pâte avec une quantité de matière alcaline dans une solution alcaline aqueuse pendant un certain temps et à une certaine température dépendant de la quantité de matière alcaline pour obtenir une répartition pratiquement uniforme de la matière alcaline dans la pâte;
l'augmentation de la consistance après l'achèvement de l'étape de traitement; et
la soumission de la pâte ayant une consistance augmentée et comprenant de la matière alcaline à un traitement d'extraction oxygène-lignine pour une grande consistance afin de réaliser une pâte partiellement libre de lignine.

27. Procédé selon la revendication 11, la viscosité de ladite pâte pratiquement libre de lignine étant maintenue à une valeur plus élevée que 10 cps.

28. Procédé selon la revendication 27, ladite pâte pratiquement libre de lignine étant maintenue à une diminution de viscosité d'environ 30 p.c. ou moins de la viscosité de ladite pâte pratiquement libre de lignine.

29. Procédé selon la revendication 11, l'étape d'extraction ultérieure de lignine comprenant en outre:
l'augmentation de la consistance de ladite pâte partiellement libre de lignine;
le broyage de la pâte ayant une consistance augmentée à une dimension de particules prédéterminée; et
la mise en contact régulière de la pâte contenant des particules réduites avec ladite quantité effective d'ozone, lorsque la pâte avance au cours du procédé.

30. Procédé selon la revendication 29, la dimension des particules de la pâte ayant une consistance augmentée étant réduite d'une telle manière qu'un contact uniforme avec l'ozone est facilité sans provoquer une détérioration importante des composants de cellulose dans la pâte.

31. Procédé selon la revendication 30, la pâte étant broyée à environ 5 mm et parcourant le procédé d'une telle manière qu'on évite un traitement inégal de la pâte par l'ozone.

32. Procédé selon la revendication 31, la pâte broyée coulant dans le même sens que l'ozone.

33. Procédé selon la revendication 31, la pâte broyée coulant à contre-courant de l'ozone.

34. Procédé selon la revendication 14, la pâte pratiquement libre de lignine étant blanchie avec du dioxyde de chlore.

35. Procédé selon la revendication 14, la pâte pratiquement libre de lignine étant blanchie avec un peroxyde.

36. Procédé selon la revendication 34 ou 35, le blanchiment augmentant le degré de blancheur GE de ladite pâte pratiquement libre de lignine à au moins 70 p.c. environ.

37. Procédé selon la revendication 34 ou 35, le traitement de blanchiment augmentant le degré de blancheur GE de la pâte pratiquement libre de lignine à au moins 80 p.c. environ.

38. Procédé selon la revendication 34 ou 35, le traitement de blanchiment augmentant le degré de blancheur GE de ladite pâte pratiquement libre de lignine à au moins 90 p.c. environ.

39. Procédé selon la revendication 1, la pâte obtenue par une extraction oxygène-lignine ayant un n° K d'environ 10 ou moins et une viscosité plus élevée qu'environ 13 cps après l'extraction oxygène-lignine, et la pâte obtenue par l'extraction ozone-lignine ayant un n° K d'environ 5 ou moins et une viscosité plus élevée qu'environ 10 et un degré de blancheur GE d'au moins 50 p.c. environ après l'extraction ozone-lignine.

40. Procédé selon la revendication 39, la matière de lignine-cellulose étant un "softwood" et étant soumise à une extraction partielle de lignine, jusqu'à ce que la pâte ait un n° K d'environ 7 à 10 et une viscosité plus élevée que 13 environ, avant l'extraction de lignine avec de l'ozone.

41. Procédé selon la revendication 40, la pâte de "softwood" ayant un n° K d'environ 3 à 4, une viscosité plus élevée qu'environ 10 et un degré de blancheur GE d'au moins 50 p.c. environ après l'extraction ultérieure de lignine avec de l'ozone.

42. Procédé selon la revendication 39, la matière de lignine-cellulose étant un "hardwood" et étant libérée partiellement de lignine jusqu'à une pâte avec un n° K d'environ 5 à 8 et une viscosité plus élevée que 13 environ, avant l'extraction ultérieure de lignine avec de l'ozone.

43. Procédé selon la revendication 42, la pâte de "hardwood" ayant un n° K d'environ 3 à 4, une viscosité plus élevée qu'environ 10 et un degré de blancheur GE d'au moins 55 p.c. environ après l'extraction ultérieure de lignine avec de l'ozone.

44. Procédé selon la revendication 39, comprenant ensuite:
la combinaison d'une pâte pratiquement libérée de lignine avec une quantité effective d'une matière alcaline dans une solution alcaline aqueuse pendant un certain temps et à une certaine température dépendant de la quantité totale de matière alcaline, pour dissoudre une partie considérable de la lignine restée dans la pâte, et d'extraire ensuite une partie de la solution alcaline aqueuse pour éliminer ainsi de la pâte pratiquement toute la lignine déjà dissoute et pour réaliser une pâte pratiquement libre de lignine.

45. Procédé selon la revendication 44, ladite étape d'extraction augmentant le degré de blancheur de la pâte d'environ 2 p.c.

46. Procédé selon la revendication 44, comprenant ensuite le blanchiment de la pâte pratiquement libre de lignine avec du dioxyde de chlore ou un peroxyde pour augmenter le degré de blancheur GE à au moins 70 p.c.

47. Procédé selon la revendication 46, le degré de blancheur GE étant augmenté à au moins 80 p.c. environ.

48. Procédé selon la revendication 46, le degré de blancheur GE étant augmenté à au moins 90 p.c. environ.

49. Procédé selon la revendication 44, la matière de lignine-cellulose étant libérée partiellement de lignine par un traitement d'extraction oxygène-lignine.

50. Procédé selon la revendication 49, le traitement d'extraction oxygène-lignine étant effectué sur une pâte de moyenne consistance.

51. Procédé selon la revendication 44, la matière de lignine-cellulose étant libérée partiellement de lignine par:
la formation d'une pâte ayant une consistance relativement petite de moins de 10 p.c. en poids;
le traitement de la pâte ayant une petite consistance avec une quantité de matière alcaline dans une solution alcaline aqueuse pendant un certain temps et à une certaine température dépendant de la quantité de matière alcaline jusqu'à obtenir une répartition pratiquement complète et en grande partie égale de la matière alcaline dans la pâte;
l'augmentation de la consistance de la pâte jusqu'à au moins 20 p.c. en poids après l'achèvement de l'étape du traitement; et
la soumission de la pâte ayant une consistance augmentée et comprenant de la matière alcaline à un traitement d'extraction oxygène-lignine pour une consistance augmentée afin d'obtenir une pâte partiellement libre de lignine avec un n° K d'environ 9 ou moins et une viscosité d'environ 13 ou plus.

52. Procédé selon la revendication 1, l'étape d'extraction oxygène-lignine comprenant:
la réduction de la consistance de la pâte à une consistance de moins de 10 p.c. en poids;
le traitement de la pâte ayant une consistance réduite avec une quantité de matière alcaline dans une solution alcaline aqueuse pendant un certain temps et à une certaine température dépendant de la quantité de matière alcaline afin de réaliser ainsi une répartition pratiquement uniforme de la matière alcaline dans la pâte;
l'augmentation de la consistance de la pâte jusqu'à au moins environ 20 p.c. en poids après l'achèvement de l'étape de traitement; et
la soumission de la pâte ayant une consistance augmentée et comprenant de la matière alcaline à un traitement d'extraction oxygène-lignine pour une consistance augmentée afin de réaliser ainsi une pâte partiellement libérée de lignine et avec un n° K d'environ 9 ou moins et une viscosité de plus de 13 cps environ;
la fourniture par l'étape d'extraction oxygène-lignine d'une pâte considérablement libérée de lignine ayant un n° K d'environ 5 ou moins, une viscosité de plus d'environ 10 et un degré de blancheur GE d'au moins 50 p.c. environ;
le procédé comprenant ensuite:
la combinaison de la pâte libérée de lignine par de l'ozone avec une quantité effective d'une matière alcaline dans une solution alcaline aqueuse pendant un certain temps et à une certaine température dépendant de la quantité totale de matière alcaline, pour dissoudre une partie considérable de la lignine éventuellement restée dans la pâte;
l'extraction d'une partie de la solution aqueuse pour éliminer ainsi de la pâte pratiquement toute la lignine déjà dissoute et pour réaliser une pâte pratiquement libre de lignine; et
le blanchiment de la pâte pratiquement libre de lignine pour augmenter le degré de blancheur GE à au moins 70 p.c. environ.

53. Procédé selon la revendication 52, le degré de blancheur GE étant augmenté à au moins 80 p.c.

54. Procédé selon la revendication 52, le degré de blancheur GE étant augmenté à au moins 90 p.c. environ.

55. Procédé selon la revendication 52, la matière de lignine-cellulose étant un "softwood" et étant libérée partiellement de lignine jusqu'à un n° K d'environ 8 à 9 et à une viscosité plus élevée qu'environ 14, avant l'extraction ultérieure de lignine avec de l'ozone.

56. Procédé selon la revendication 55, le "softwood" ayant un n° K entre environ 3 et 4, une viscosité d'environ 10 et un degré de blancheur GE d'au moins 54 p.c. environ après l'extraction ultérieure avec de l'ozone.

57. Procédé selon la revendication 52, la matière de lignine-cellulose étant un "hardwood" et étant libérée partiellement de lignine jusqu'à un n° K d'environ 6 à 7 et à une viscosité plus élevée qu'environ 15, avant que l'extraction ultérieure de lignine avec de l'ozone ait lieu.

58. Procédé selon la revendication 57, la pâte de "hardwood" ayant un n° K entre environ 3 et 4, une viscosité plus élevée qu'environ 10 et un degré de blancheur GE d'au moins 63 p.c. environ, après ladite étape d'extraction de lignine avec de l'ozone.

59. Procédé selon la revendication 52, la matière de lignine-cellulose partiellement libérée de lignine étant obtenue par une trituration Kraft, une trituration Kraft AQ ou une étape d'extraction de lignine prolongée d'une matière de lignine-cellulose.

60. Procédé selon la revendication 52, comprenant la diminution du n° K de la pâte ayant une consistance d'environ 60 p.c. pendant l'étape d'extraction oxygène-lignine sans détériorer considérablement les composants de cellulose de la pâte.

61. Procédé selon la revendication 52, la pâte étant soumise à une étape d'extraction oxygène-lignine lorsqu'elle a une grande consistance sans changer dans une large mesure la viscosité de la pâte.

62. Procédé selon la revendication 52, comprenant la diminution du n° K d'environ 25 p.c.par rapport à la viscosité de la pâte pendant l'étape d'extraction oxygène-lignine.

63. Procédé selon la revendication 52, la consistance de la pâte, laquelle a été traitée avec la solution alcaline aqueuse avant l'étape d'extraction oxygène-lignine, est comprise entre environ 1 et 4,5 p.c. en poids.

64. Procédé selon la revendication 52, la consistance de la pâte étant augmentée à environ 25 à 35 p.c. en poids, l'exécution de l'étape d'extraction oxygène-lignine.

65. Procédé selon la revendication 52, la quantité de matière alcaline répartie dans la pâte ayant une petite consistance avant l'extraction oxygène-lignine est comprise entre environ 15 et 30 p.c. en poids par rapport au poids sec de la pâte.

66. Procédé selon la revendication 65, la solution alcaline aqueuse ayant une concentration de matière alcaline comprise entre environ 20 et 120 g/l, de sorte que la concentration de la matière alcaline dans la pâte ayant une petite consistance est comprise entre 6,5 et 13 g/l.

67. Procédé selon la revendication 52, l'étape de traitement alcaline étant effectuée pendant un temps compris entre 1 et 15 min. environ et à une température comprise entre 90 et 150°F environ.

68. Procédé selon la revendication 52, la pâte formée à l'origine étant une pâte "brownstock", et lors de l'étape pour l'augmentation de la consistance de la pâte, au moins une partie du liquide obtenu de la solution alcaline étant ensuite reconduite à l'étape de traitement alcaline.

69. Procédé selon la revendication 1:
la pâte étant formée à l'origine comme une pâte "brownstock" avec un n° K compris entre environ 10 et 24 par une trituration Kraft, une trituration Kraft AQ ou une extraction de lignine prolongée de la matière de lignine-cellulose;
l'étape d'extraction oxygène-lignine comprenant:
la diminution de la consistance de ladite pâte à environ 1 à 4,5 p.c. en poids;
le traitement de la pâte ayant une consistance réduite avec une quantité de matière alcaline dans une solution alcaline aqueuse ayant une concentration de la matière alcaline comprise entre environ 20 et 120 g/l pendant un temps compris entre environ 1 et 15 minutes et une température comprise entre environ 90 et 150°F, de telle sorte que la concentration de la matière alcaline dans la pâte ayant une consistance réduite est comprise entre environ 6,5 et 13 g/l pendant cette étape de traitement, pour achever ainsi une répartition pratiquement uniforme de la matière alcaline dans la pâte;
l'augmentation de la consistance de la pâte traitée avec un alcalin à environ 25 à 35 p.c. en poids;
la soumission de la pâte ayant une consistance augmentée à une extraction oxygène-lignine pour une grande consistance sans changer dans une large mesure la viscosité de la pâte et afin de réaliser ainsi une pâte partiellement libre de lignine et avec un n° K d'environ 10 ou moins et une viscosité plus élevée qu'environ 13, le rapport entre le n°de K et la viscosité de ladite pâte étant diminué d'au moins 25 p.c. pendant l'extraction oxygène-lignine;
l'étape d'extraction oxygène-lignine fournissant une pâte en grande partie libre de lignine et avec un n° K d'environ 5 ou moins, une viscosité plus élevée qu'environ 10 et un degré de blancheur GE d'au moins 50 p.c. environ;
le procédé comprenant ensuite:
la combinaison de la pâte en grande partie libre de lignine avec une quantité effective d'une matière alcaline dans une solution alcaline aqueuse pendant un certain temps et à une certaine température dépendant de la quantité de matière alcaline, pour dissoudre une partie considérable de la lignine restée dans la pâte;
l'extraction d'une partie de la solution aqueuse pour éliminer ainsi de la pâte pratiquement toute la lignine déjà dissoute et pour réaliser une pâte pratiquement libre de lignine; et
le blanchiment de la pâte pratiquement libre de lignine pour augmenter le degré de blancheur GE à au moins 70 p.c. environ.

70. Procédé selon la revendication 69, le degré de blancheur GE étant augmenté à au moins 80 p.c. environ.

71. Procédé selon la revendication 69, le degré de blancheur GE étant augmenté à au moins 90 p.c. environ

72. Procédé selon la revendication 69, comprenant la diminution du n° K de la pâte ayant une consistance augmentée d'environ 60 p.c. pendant l'étape d'extraction oxygène-lignine sans détériorer dans une large mesure les composants de cellulose de la pâte.

73. Procédé selon la revendication 69, la pâte pratiquement libre de lignine étant blanchie avec du dioxyde de chlore ou un peroxyde.

74. Procédé selon la revendication 73, le peroxyde étant un peroxyde d'hydrogène.

75. Procédé selon la revendication 69, comprenant ensuite l'addition à la pâte d'un agent chélateur avant l'étape d'extraction oxygène-lignine, afin de rendre les ions métalliques pratiquement non réactifs par rapport à l'ozone.

76. Procédé selon la revendication 75, l'agent chélateur étant du ADTP, de l'AEDT ou de l'acide oxalique.

77. Procédé selon la revendication 69, comprenant ensuite le réglage du pH de la pâte jusque dans une plage de 1 à 4 en ajoutant à la pâte une quantité suffisante de matière acide, avant l'étape d'extraction ozone-lignine.

78. Procédé selon la revendication 69, comprenant ensuite l'augmentation de la consistance à une valeur comprise entre environ 25 et 50 p.c. en poids, avant l'étape d'extraction ozone-lignine.

79. Procédé selon la revendication 78, la consistance de la pâte étant augmentée à une valeur comprise entre environ 35 et 45 p.c. en poids, avant l'étape d'extraction ozone-lignine.

80. Procédé selon la revendication 69, comprenant le broyage de la pâte à un diamètre plus petite qu'environ 5 mm après l'étape d'extraction oxygène-lignine et avant l'étape d'extraction ozone-lignine.

81. Procédé selon la revendication 69, comprenant ensuite la maintenance de la pâte à une température de moins d'environ 120°F pendant l'étape d'extraction ozone-lignine.

82. Procédé selon la revendication 69, l'ozone étant fourni par un mélange comprenant de l'ozone et de l'oxygène.

83. Procédé selon la revendication 82, la concentration d'ozone dans le mélange étant comprise entre environ 1 et 8 p.c. en volume.

84. Procédé selon la revendication 69, l'ozone étant fourni par un mélange d'ozone et d'air.

85. Procédé selon la revendication 84, la concentration d'ozone étant comprise entre environ 1 et 4 p.c. en volume.

86. Procédé selon la revendication 69, comprenant le transport de la pâte partiellement libre de lignine pendant l'étape d'extraction ozone-lignine, de telle sorte que pratiquement toute la pâte est exposée à l'ozone.

87. Procédé selon la revendication 86, l'ozone étant ajouté à contre-courant de la pâte avançante.

88. Procédé selon la revendication 86, l'ozone étant ajouté dans le même sens que la pâte avançante.

89. Procédé selon la revendication 1:
la pâte libérée de lignine par l'ozone ayant un n° K d'environ 10 ou moins et une viscosité plus élevée qu'environ 13 cps;
l'étape d'extraction ozone-lignine comprenant:
l'addition à la pâte d'un agent chélateur pour rendre les ions métalliques de la pâte pratiquement non réactifs par rapport à l'ozone;
le réglage du pH de ladite pâte jusque dans une plage d'environ 1 à 4, en ajoutant une quantité suffisante de matière acide;
l'augmentation de la consistance de ladite pâte jusqu'à une valeur comprise entre environ 25 et 50 p.c.;
le broyage de la pâte ayant une consistance augmentée à un diamètre de moins d'environ 5 mm; et
l'extraction de lignine de ladite pâte ayant une consistance augmentée avec une quantité effective d'ozone pendant un temps suffisamment long en transportant la pâte broyée d'une telle manière que pratiquement toute la pâte est exposée à l'ozone, afin d'obtenir une pâte qui comprend considérablement moins de lignine et qui a un n° K d'environ 5 ou moins, une viscosité plus élevée qu'environ 10 et un degré de blancheur d'au moins 50 p.c. environ;
lequel procédé comprend ensuite:
la combinaison de la pâte en grande partie libre de lignine avec une quantité effective d'une matière alcaline dans une solution alcaline aqueuse pendant un certain temps et à une certaine température dépendant de la quantité de matière alcaline, pour dissoudre une partie considérable de la lignine éventuellement restée dans la pâte;
l'extraction d'une partie de la solution alcaline aqueuse pour éliminer ainsi de la pâte pratiquement toute la lignine déjà dissoute et pour réaliser une pâte pratiquement libre de lignine; et
le blanchiment de la pâte pratiquement libre de lignine avec du dioxyde de chlore pour augmenter son degré de blancheur GE à au moins 70 p.c. environ.

90. Procédé selon la revendication 89, le degré de blancheur GE étant augmenté à au moins 80 p.c. environ.

91. Procédé selon la revendication 89, le degré de blancheur GE étant augmenté à au moins 90 p.c. environ.

92. Procédé selon la revendication 89, l'étape de trituration comprenant une trituration Kraft et l'étape d'extraction oxygène-lignine diminuant le n° K de la pâte d'environ 60 p.c. au moins sans détériorer considérablement les composants de cellulose de la pâte et sans réellement changer la viscosité de la pâte.

93. Procédé selon la revendication 92, l'étape de trituration comprenant une trituration Kraft AQ.

94. Procédé selon la revendication 93, l'étape d'extraction oxygène-lignine diminuant le n° K de la pâte d'environ 60 p.c. au moins sans détériorer dans une large mesure les composants de cellulose de la pâte et sans changer dans une large mesure la viscosité de la pâte.

95. Procédé selon la revendication 89, l'étape de trituration comprenant la combinaison d'une trituration Kraft et une extraction de lignine prolongée, et l'étape d'extraction oxygène-lignine diminuant le n° K de la pâte d'environ 60 p.c. au moins sans détériorer dans une large mesure les composants de cellulose de la pâte et sans changer considérablement la viscosité de la pâte.

96. Procédé selon la revendication 89, la pâte étant transportée pendant l'extraction ozone-lignine d'une telle manière que la pâte est maintenue à une température de moins d'environ 120°F.

97. Procédé selon la revendication 89, l'agent chélateur et un acide sont ajoutés à la pâte dans une chambre de mélange.

98. Procédé selon la revendication 97, au moins une partie du liquide enlevé de la pâte lors de l'étape pour l'augmentation de la consistance étant reconduite à la chambre de mélange.

99. Procédé selon la revendication 97, la pâte étant transportée dans le même sens que l'ozone.

100. Procédé selon la revendication 97, la pâte étant transportée à contre-courant de l'ozone.

101. Procédé selon la revendication 1:
la pâte libérée de lignine par de l'oxygène ayant un n° K d'environ 10 ou moins, et une viscosité plus élevée qu'environ 13 cps;
l'étape d'extraction ozone-lignine comprenant:
l'addition à la pâte d'un agent chélateur pour rendre les ions métalliques de la pâte pratiquement non réactifs par rapport à l'ozone;
le réglage du pH de ladite pâte jusque dans une plage d'environ 1 à 4, en ajoutant une quantité suffisante de matière acide;
l'augmentation de la consistance de la pâte jusqu'à une valeur comprise entre environ 25 et 50 p.c.;
le broyage de la pâte ayant une consistance augmentée à un diamètre de moins d'environ 5 mm; et
l'extraction de lignine de la pâte ayant une consistance augmentée au moyen d'une quantité effective d'ozone pendant un temps suffisamment long, afin de réaliser une pâte en grande partie libérée de lignine et avec un n° K d'environ 5 ou moins, une viscosité plus élevée qu'environ 10 et un degré de blancheur GE d'au moins 50 p.c. environ;
lequel procédé comprend ensuite:
la combinaison de la pâte dans une large mesure libérée de lignine avec une quantité effective d'une matière alcaline dans une solution alcaline aqueuse pendant un certain temps et à une certaine température dépendant de la quantité de matière alcaline, pour dissoudre une partie considérable de la lignine restée dans la pâte;
l'extraction d'une partie de la solution alcaline aqueuse pour éliminer ainsi de la pâte pratiquement toute la lignine déjà dissoute et pour réaliser une pâte pratiquement libre de lignine;
le blanchiment de la pâte pratiquement libre de lignine avec un peroxyde pour augmenter son degré de blancheur GE à au moins 70 p.c. environ.

102. Procédé selon la revendication 101, le degré de blancheur GE étant augmenté à au moins 80 p.c. environ.

103. Procédé selon la revendication 101, le degré de blancheur GE étant augmenté à au moins 90 p.c. environ.

104. Procédé selon la revendication 101, l'étape de trituration comprenant une trituration Kraft et l'étape d'extraction oxygène-lignine diminuant le n° K de la pâte d'au moins 60 p.c. sans détériorer considérablement les composants de cellulose de la pâte et sans considérablement changer sa viscosité.

105. Procédé selon la revendication 101, l'étape de trituration comprenant une trituration Kraft AQ.

106. Procédé selon la revendication 105, l'étape d'extraction oxygène-lignine diminuant le n° K de la pâte d'au moins 60 p.c. sans détériorer considérablement les composants de cellulose de la pâte et sans changer considérablement la viscosité de la pâte.

107. Procédé selon la revendication 101, l'étape de trituration comprenant la combinaison d'une trituration Kraft AQ et une extraction de lignine prolongée, et l'étape d'extraction oxygène-lignine diminuant le n° K de la pâte d'au moins 60 p.c. sans détériorer dans une large mesure les composants de cellulose de la pâte et sans changer dans une large mesure la viscosité de la pâte.

108. Procédé selon la revendication 89 ou 101, l'étape d'extraction ozone-lignine diminuant le n° K de la pâte d'au moins 50 p.c.

109. Procédé selon la revendication 89 ou 101, l'étape de blanchiment augmentant le degré de blancheur GE de la pâte d'au moins 50 p.c.

110. Procédé selon la revendication 109, le degré de blancheur GE de la pâte étant augmenté d'au moins 83 p.c.

111. Procédé selon la revendication 1:
la pâte étant lavée entre l'étape de décomposition chimique et l'étape d'extraction oxygène-lignine, la pâte ayant un n° K d'environ 10 ou moins et un viscosité plus élevée qu'environ 13 cps après l'étape d'extraction oxygène-lignine;
le procédé comprenant ensuite:
le lavage de la pâte libérée de lignine par de l'oxygène;
la continuation de l'étape d'extraction ozone-lignine pour obtenir une pâte considérablement libérée de lignine et avec un n° K d'environ 5 ou moins, une viscosité plus élevée qu'environ 10 et un degré de blancheur GE d'environ 50 p.c. au moins;
le lavage de la pâte dans une large mesure libérée de lignine;
la combinaison de la pâte dans une large mesure libérée de lignine avec une quantité effective d'une matière alcaline dans une solution alcaline aqueuse pendant un certain temps et à une certaine température dépendant de la quantité de matière alcaline, pour dissoudre une partie considérable de la lignine éventuellement restée dans la pâte;
l'extraction d'une partie de la solution alcaline aqueuse pour éliminer ainsi de la pâte pratiquement toute la lignine déjà dissoute et pour former une pâte réellement libre de lignine;
le lavage de la pâte réellement libre de lignine;
le blanchiment de la pâte réellement libre de lignine avec du dioxyde de chlore ou un peroxyde pour augmenter son degré de blancheur GE à au moins 70 p.c. environ; et
le lavage de la pâte blanchie.

112. Procédé selon la revendication 111, le degré de blancheur GE étant augmenté à au moins 80 p.c. environ.

113. Procédé selon la revendication 111, le degré de blancheur GE étant augmenté à au moins 90 p.c. environ.

114. Procédé selon la revendication 111, le traitement de lavage pour le blanchiment de la pâte comprenant: le lavage de la pâte avec de l'eau fraîche et l'enlèvement de la pâte de la lavure qui s'écoule.

115. Procédé selon la revendication 111, du dioxyde de chlore étant utilisé lors de l'étape de blanchiment et la lavure d'écoulement provenant de la pâte étant évacuée.

116. Procédé selon la revendication 111, du dioxyde de chlore étant utilisé lors du traitement de blanchiment et la lavure s'écoulant de la pâte blanchie étant traitée par une osmose inversée pour former un filtrat traité, au moins une partie du filtrat formé étant conduit au traitement de lavage de la pâte pratiquement libre de lignine.

117. Procédé selon la revendication 111, un peroxyde étant utilisé lors du traitement de blanchiment et au moins une partie de la pâte blanchie étant reconduite à l'étape de lavage de la pâte pratiquement libre de lignine.

118. Procédé selon la revendication 116 ou 117, le traitement de lavage de la pâte pratiquement libre de lignine comprenant: le lavage de la pâte avec de la lavure provenant de la pâte pratiquement libre de lignine et l'enlèvement de la pâte de la lavure résultante et le retour d'au moins une partie de ladite lavure au traitement de lavage de la pâte pratiquement libre de lignine.

119. Procédé selon la revendication 118, le traitement de lavage de la pâte pratiquement libre de lignine comprenant: le lavage de ladite pâte avec la lavure provenant de la pâte en grande partie libérée de lignine, l'enlèvement de la pâte de la lavure résultante, et l'addition d'au moins une partie de cette lavure au traitement de lavage de la pâte partiellement libérée de lignine.

120. Procédé selon la revendication 119, le traitement de lavage de la pâte partiellement libérée de lignine comprenant: le lavage de ladite pâte avec de la lavure provenant de la pâte en grande partie libérée de lignine, l'enlèvement de la pâte de la lavure résultante, et l'addition d'au moins une partie de ladite lavure au traitement de lavage de la pâte.

121. Procédé selon la revendication 120, le traitement de lavage de la pâte comprenant: le lavage de ladite pâte avec de la lavure provenant de la pâte partiellement libérée de lignine, l'enlèvement de la pâte de la lavure résultante, et l'accumulation et la concentration de ladite lavure pour combustion dans un chauffe-eau de récupération.

122. Procédé selon la revendication 111 ou 121, du dioxyde de chlore avec une teneur minimale en chlore étant utilisé pour la traitement de blanchiment.

123. Procédé selon la revendication 111 ou 121, la quantité d'eau nécessaire pour les traitements de lavage étant réduite considérablement par rapport aux procédés connus de CEDED ou OC/DED.

124. Procédé selon la revendication 115, le liquide d'écoulement ayant une couleur qui n'est pas plus forte qu'environ 2 livres par tonne, un BOD5 qui n'est pas plus grand qu'environ 2 livres par tonne et une quantité totale de chlorures organiques qui n'est pas plus grande que 2 environ.

125. Procédé selon la revendication 75, l'agent chélateur étant un polycarboxylate ou un dérivé de polycarboxylate.

126. Procédé selon la revendication 75, l'agent chélateur étant utilisé en une quantité de 0,1 à 0,2 p.c. en poids par rapport au poids sec à l'étuve de la pâte.

127. Procédé selon la revendication 75, la pâte étant acidifiée jusqu'à un pH compris entre environ 1 et 4 avant le traitement avec l'agent chélateur.

128. Procédé selon la revendication 75, le degré de blancheur de la pâte étant augmenté avec un peroxyde après le traitement de blanchiment avec de l'ozone.
